# EUROPEAN PATENT SPECIFICATION

(11) **EP 0 680 521 B1**
(45) Date of publication and mention of the grant of the patent: **14.03.2001**
(21) Application number: 94900231.5
(22) Date of filing: 19.11.1993
(51) Int. Cl.: C22C 1/10, B22F 1/02, C22C 32/00, C21C 7/00

(54) **FERROUS METAL ALLOYS, IN PARTICULAR FOR CASTING ROLLING MILL ROLLS**
EISENMETALLGUSSWERKSTOFFE, INSBESONDERE FÜR WALZROLLEN
METAUX FERREUX COULES, EN PARTICULIER POUR CYLINDRES DE LAMINAGE

(30) Priority: 19.11.1992 GB 9224271; 23.07.1993 GB 9315356
(43) Date of publication of application: 08.11.1995
(73) Proprietor: SHEFFIELD FORGEMASTERS LIMITED, Sheffield, South Yorkshire S9 2WZ (GB)
(72) Inventor: WRAGG, David, Cheshire CW1 1LH (GB); HEWITT, Paul Herbert, Steel Hexham NE47 0HA (GB); NUTTING, Jack, Leeds LS16 5NP (GB)
(74) Representative: Leach, John Nigel
(86) International application number: GB9302380
(87) International publication number: WO9411541

(56) References cited:
- EP-A- 0 123 961
- EP-A- 0 386 515
- EP-A- 0 550 725
- WO-A-91/16466
- CH-A- 473 068
- US-A- 5 023 145

## Description

This invention relates to cast iron or steel, herein defined as "engineering ferrous metals". More particularly, this invention relates to a rolling mill roll comprising cast iron or steel.

Mechanical properties of engineering ferrous metals and hence a rolling mill roll made of engineering ferrous metals are influenced by the presence of carbides whose distribution and formation is dependent upon carbon content, heat treatment and the addition of other alloying elements. Carbon is added to engineering ferrous metals whilst the cast iron or steel is molten and the carbon is subsequently precipitated as metal carbides during solidification and during phase transformation in the solid state. Such carbides are referred to herein as "transformation carbides". Thus, the type and the amount of transformation carbide present in engineering ferrous metals is limited by the thermo-dynamics and chemistry of a particular ferrous metal and are represented by the relevant phase diagram.

There has been a long standing desire to provide carbides of different composition and volume fraction in engineering ferrous metals than is possible by the previously known techniques described above which rely on phase transformation as the metal cools from liquid state.

US-A-5,023,145 discloses an alloy having a substantially uniform distribution of three carbide aggregates in which a uniform distribution of the three carbides is achieved by using a relatively heavier binder material with a relatively lighter carbide rendering the resultant aggregates relatively similar in density.

EP-A-0386515 discloses a process for manufacture of a metallic compound body using an electro slag refining process in the course of which solid alloy-carbide particles in the form of tungsten carbide are added to the melt.

WO 91/16466 discloses an iron based alloy having dispersed therein tungsten carbide particles.

WO 93/03192 discloses adding, to an iron based melt, iron-coated alloy carbide particles (WTiC) of matching density (7 to 7.9g/cm³.

An object of the invention is to provide a new and improved method of making an engineering ferrous metal whereby the above mentioned problems are overcome or are reduced and a further object of the invention is to provide a new and improved engineering ferrous metal product having a desired carbide content which is not limited by thermo-dynamic considerations.

According to one aspect of the invention we provide a method according to claim 1.

By "wetting" we mean the ability of the liquid engineering ferrous metal to wet the coating metal. More particularly, for example, where the interfacial tension between the liquid engineering ferrous metal and the solid coating metal is such that the contact angle there between is 0° - 90°.

By "a density which matches" we mean a density lying in the range 6-8 gms per cc. This is to be compared with a typical density of 7 gms per cc. for cast iron and steel. More preferably, the alloy carbide particles have a density of ± 5% of the density of the engineering ferrous metal to which they are added.

The weltability of the coated particles and the density of the alloy carbide particles each promote a uniform distribution of the carbide particles in the liquid engineering ferrous metal which is retained when the metal solidifies.

By a "uniform distribution" we mean an even distribution throughout the section of a casting made of the engineering ferrous metal with no significant segregation. The solid carbide particles are not orientated in any direction and are distributed across all phases of the micro-structure.

The coating metal preferably comprises iron or an iron carbon alloy, but may comprise an alloy of two or more elements selected from the group comprising iron, nickel, copper, titanium and carbon, or may be nickel or copper and usual incidentals.

The coating metal may comprise nitrogen, for example up to about 0.1% nitrogen.

If the coating is iron, then because iron has a higher melting point than the engineering ferrous metal to which it is to be added, which would inhibit wettability, it is preferred to add an appropriate amount of at least one alloying element such as carbon, nickel, copper or titanium to the iron to produce an alloy having a melting point which matches the operating temperature of the ferrous metal. By "matches" we mean that the melting point of the coating and said operating temperature are preferably within approximately 20 - 30°C of each other.

The term "operating temperature" is defined herein as the temperature of the engineering ferrous metal at which the coated carbide particles are added.

The iron coating may contain up to 3.5% carbon.

If the alloy carbide particles are coated with iron or with an iron alloy having a lower carbon content than that of the engineering ferrous metal to which they are added the coated alloy carbide particles may be added to the engineering ferrous metal and permitted to dwell therein sufficiently long for carbon from the engineering ferrous metal to diffuse into the coating and so produce a composition which has a melting point which matches the operating temperature of engineering ferrous metal.

It is particularly preferred that the carbide particles have a matching density as described above when the particles are left in the molten engineering ferrous metal for a dwell time long enough for carbon to diffuse into the coating to cause the melting points to match.

If desired, the composition of the coating metal may be such as to provide a melting point which is more than 30°C below the operating temperature of the engineering ferrous metal to which the coated particles are added.

The coated alloy carbide particles may be added to the liquid engineering ferrous metal either in the melting furnace or in a ladle into which the metal has been poured from the melting furnace, or in the stream of metal being poured from the melting furnace to the ladle, or in the stream of metal being poured from the ladle into a mould.

It is preferred to add the coated alloy carbide particles in the melting furnace so as to maximise the dwell time of the alloy carbide particles in the ferrous metal prior to the onset of solidification.

It is particularly preferred that the melting furnace is an induction furnace, since an induction furnace provides good stirring of the melt.

We have found that the titanium of the carbide oxidises to form titanium oxide which can react with silicon from the furnace lining to form a hard crust on the metal surface which may entrap the carbide particles and reduce their distribution in the molten metal.

The coated alloy carbide particles may be added to the ferrous engineering metal melt in the form of a powder comprising powder particles having a particle size up to 2mm and preferably of about 500 micro-meters (microns) and containing alloy carbide particles having a particle size of up to 10 micro-meters (microns) and preferably in the range 1-5 micro-meters (microns) and more preferably 2-5 micro-meters (microns).

The powder particles may comprise:-

| | |
|---|---|
| 25% | coating metal. |
| 30% | Ti |
| 35% | W |
| Balance | Carbon (including up to 3.5% free carbon) and usual incidentals. |

The coating metal may comprise iron such as alpha iron and may comprise wholly or substantially wholly alpha iron and up to 3.5% free carbon.

Such a coating metal has a melting point of about 1520°C and hence the powder is suitable for adding to engineering ferrous metal having an operating temperature of about 1500°C or above.

Alternatively the coating metal may comprise an alloy of iron, nickel and carbon.

In this case the powder and alloy carbide particles may be of the same size as mentioned above and the powder particles may comprise:-

| | |
|---|---|
| 27% | coating metal. |
| 30% | Ti |
| 35% | W |
| Balance | Carbon (including up to 0.5% free carbon) and usual incidentals. |

The coating material may comprise an alloy of iron, nickel and carbon:

| | |
|---|---|
| 59% | nickel |
| 41% | iron and up to 0.5% free carbon and usual incidentals. |

Such a coating metal has a melting point of about 1420°C and is particularly suitable for adding to engineering ferrous metals having an operating temperature of below about 1500°C.

If powder having an alpha iron matrix is added to metal having such a relatively low operating temperature, it is found that the powder may not break down enough at the temperature of the melt for best distribution of the alloy carbide particles in the melt. With such engineering ferrous metal compositions it is not possible to increase the temperature of the melt because the iron tends to become a "white" iron as a result of superheat inhibiting the formation of graphite. White iron is unsuitable for use as a roll material.

If desired, the coating metal may be an alloy of either iron, nickel and copper or iron and copper with or without carbon in each case to provide a lower melting point.

Where the coating metal contains significant amounts of carbon, for example, 2 - 3.5%, it has been found that the product to which the powder has been added is softer than expected because more graphite is transformed in the metal. It is believed that this is due to the free carbon in the relatively fine powder particles acting as an inoculant. Accordingly the carbon content of the powder is preferably reduced to less than about 0.5% in order to minimise the softening effect.

However, where the product is a roll used in an application where spalling due to cycles of reversed thermal stress is likely, it may be desirable to increase the amount of graphite in the product since graphite provides a better thermal resistance and hence resistance to spalling.

Where the coating metal contains nickel a similar softening effect can occur even though the coating metal has relatively low carbon, e.g. 0.5%. This softening effect can be overcome or reduced by adjusting the chemical composition of the engineering ferrous metal.

Alternatively the coated alloy carbide particles may he added during an electroslag remelting operation.

According to a second aspect of the present invention we provide an engineering ferrous metal product according to claim 22.

The microstructure may comprise matrix and carbide which have resulted from phase transformation of the engineering ferrous metal; said carbide being referred to herein, as mentioned hereinbefore, as "transformation carbide".

The discrete alloy carbide particles preferably have a higher hardness than the transformation carbide present in the microstructure.

The discrete alloy carbide particles may increase the hardness of the engineering ferrous metal by virtue of the law of mixtures and/or the phase transformation of the engineering ferrous metal may be modified and enhanced by the presence of the discrete alloy carbide particles.

The discrete alloy carbide particles may be distributed in the matrix and/or the transformation carbide.

The discrete alloy carbide particles may be uniformly distributed in the microstructure.

In both the first and the second aspects of the invention:-

The alloy carbide particles may have a hardness of about 3,000 vpn.

The alloy carbide is preferably selected from the group comprising chromium, molybdenum, titanium, tungsten, niobium, vanadium or mixed carbides thereof such as Cr₇C₃, (CrMo)₇C₃ or mixed carbo-nitrides.

For example, the carbide may be a mixed tungsten titanium carbide of the kind (TiW)C where the ratio of titanium to tungsten is about 1:1 by weight.

The alloy carbide may comprise Ti and W in the ratio range:
1:1 to 1:1.17

The alloy carbide may contain nitrogen, for example up to about 0.1% nitrogen.

The alloy carbide preferably comprises:-

| | |
|---|---|
| 42% | Ti |
| 49% | W |
| 9% | C ans usual residuals |

The alloy carbide may contain up to 0.1% nitrogen.

The alloy carbide particles have a very low co-efficient of thermal expansion compared to the co-efficient of thermal expansion of engineering ferrous metals. Accordingly, if relatively large alloy carbide particles were present in the engineering ferrous metals this would give rise to high stresses on cooling, causing dislocations to form, and leading to thermal fatigue.

The alloy carbide particles preferably have a maximum dimension of up to 10 microns and preferably 1-5 microns and more preferably 2-5 microns.

The amount of alloy carbide particles added is such as to achieve up to 20% by volume of alloy carbide particles in the solid metal. Generally, the alloy carbide content may be in the range 0.1 to 20% by volume, and may be in the range 1 to *20%* and more preferably 3 to 10% when a hardening effect based on the law of mixtures is provided. However, the alloy carbide content may be lower, e.g. down, for example from about 1%, to about 0.5% or 0.1% or less when a hardening effect based on a modification of the transformation of the microstructure is provided.

The engineering ferrous metal preferably has a carbon content lying in the range 0.3 - 3.8%.

The engineering ferrous metals may contain chromium and may have a chromium content which is greater than or equal to 1%.

The engineering ferrous metal may contain nitrogen, for example up to 0.1% nitrogen.

Where the coating metal, and/or the alloy carbide and/or the engineering ferrous metal contains nitrogen it is considered that titanium carbonitrides may be precipitated in the microstructure of the engineering ferrous metal. The total nitrogen content of all the components may be limited to about 0.1% nitrogen.

The engineering ferrous metal may have a composition falling within one of the following ranges:

| Indefinite Chill such as: | | | | | | | |
|---|---|---|---|---|---|---|---|
| T.C. | Si | Mn | Ni | Cr | Mo | Cu | V |
| 3.00 | 0.70 | 0.40 | 3.0 | 0.8 | 0.15 | 0.10 | up to |
| 3.50 | 1.20 | 1.40 | 5.5 | 2.0 | 0.50 | 1.00 | 0.50 |

| Chromium Irons such as: | | | | | | | |
|---|---|---|---|---|---|---|---|
| T.C. | Si | Mn | Ni | Cr | Mo | Cu | V |
| 2.00 | 0.40 | 0.40 | 0.40 | 10.00 | 0.50 | 0.10 | 0.10 |
| 3.00 | 2.00 | 1.50 | 1.50 | 20.00 | 3.00 | 2.00 | 0.50 |

| High Alloy Steels such as: | | | | | | | |
|---|---|---|---|---|---|---|---|
| T.C. | Si | Mn | Ni | Cr | Mo | V | W |
| 0.50 | 0.40 | 0.40 | 0.10 | 5.00 | 0.50 | 0.00 | 0.00 |
| 1.50 | 0.80 | 1.00 | 1.00 | 15.00 | 5.00 | 5.00 | 5.00 |

| Tool Steels such as: | | | | | | | |
|---|---|---|---|---|---|---|---|
| T.C. | Si | Mn | Ni | Cr | Mo | V | W |
| 1.00 | 0.30 | 0.30 | - | 11.00 | 0.70 | 0.80 | 1.00 |
| 2.00 | 0.40 | 0.50 | - | 13.00 | 1.00 | 1.20 | 1.40 |

or

| T.C. | Si | Mn | Ni | Cr | Mo | V | W |
|---|---|---|---|---|---|---|---|
| 0.90 | 0.40 | 0.80 | 0.00 | 10.00 | 2.50 | 2.50 | 0.00 |
| 0.95 | 0.50 | 0.85 | 0.10 | 11.00 | 3.00 | 3.00 | 0.50 |

| S | P |
|---|---|
| 0.00 | 0.00 |
| 0.02 | 0.02 |

Such a steel may be used for the finishing stands, of a hot strip steel mill.

| Medium Alloy Steels such as : | | | | | | | |
|---|---|---|---|---|---|---|---|
| T.C. | Si | Mn | Ni | Cr | Mo | V | W |
| 0.30 | 0.40 | 0.40 | 0.10 | 2.00 | 0.10 | 0.10 | 0.10 |
| 1.50 | 0.80 | 1.00 | 1.00 | 5.00 | 0.50 | 0.50 | 0.50 |

| Low Alloy Steels such as: | | | | | | | |
|---|---|---|---|---|---|---|---|
| T.C. | Si | Mn | Ni | Cr | Mo | V | W |
| 0.30 | 0.40 | 0.40 | 0.10 | 0.10 | 0.10 | 0.10 | 0.10 |
| 1.50 | 0.80 | 1.00 | 1.00 | 2.00 | 0.50 | 0.50 | 0.50 |

| S.G. Irons such as: | | | | | | |
|---|---|---|---|---|---|---|
| T.C. | Si | Mn | Ni | Cr | Mo | Cu |
| 2.50 | 0.90 | 0.10 | 0.10 | 0.00 | 0.00 | 0.00 |
| 3.70 | 3.00 | 1.00 | 5.00 | 1.00 | 2.00 | 2.00 |

In all cases, iron and usual incidentals comprise the balance.

Nitrogen, for example up to 0.1%, may also be present where appropriate.

According to a third aspect of the invention we provide a rolling mill roll having at least an outer part which comprises an engineering ferrous metal according to the second aspect of the invention or an engineering ferrous metal made according to the first aspect of the invention.

According to a fourth aspect of the invention, we provide a method of making a rolling mill roll wherein a metal made according to the first aspect of the invention or according to the second aspect of the invention is cast to make at least an outer part of the rolling mill roll.

In a first alternative, the rolling mill roll may be a composite rolling mill roll of the kind having a core and an outer shell with, optionally, at least one intermediate layer, in which the shell comprises said outer part.

The alloy carbide particles may be introduced into a molten engineering ferrous metal of which the shell is to be formed and then the engineering ferrous metal with the alloy carbide particles therein may be poured into a mould.

The carbide particles may be introduced into the mould under a protective atmosphere of inert gas such as argon, or under a vacuum.

The composite roll may be made by centrifugal casting.

In a second alternative, a roll may be made by performing an electroslag remelting operation on a consumable electrode which comprises an inner body provided with an external cladding comprising a hollow element containing said coated alloy carbide particles.

The inner body may be tubular or solid.

The hollow element may comprise a sleeve or a plurality of discrete hollow elements such as tubes.

The material inside the or each hollow element may also comprise a powder alloy ingredient(s).

The powder of the alloy element may have a mesh size of less than 3mm, but may have a mesh size up to 5mm and may lie in the range 2 - 5mm.

Each hollow element or hollow sleeve may comprise steel, such as mild steel or stainless steel.

Where the cladding comprises discrete elements, at least one of the elements may be of different composition to the other elements.

The inner body may be of constant composition throughout its cross-section or it may be of varying composition across at least part of its cross-section.

The droplets of molten coated alloy carbide or of molten coated alloy carbide and alloy ingredient from the hollow elements, because of their spatial and temperature proximity to the mould wall, solidify relatively rapidly at or adjacent to the mould wall whereby the region of the re-melted ingot adjacent the mould wall has a relatively high and uniform distribution of alloy carbide or carbide and alloy ingredient. Of course, if the alloy carbide particles do not wholly melt they are trapped in the melt adjacent the mould wall as it solidifies relatively rapidly.

At or adjacent to the centre of the ingot there may be a relatively low uniform distribution of alloy carbide particles or carbide particles and alloy ingredient.

The melting point of the alloy ingredient and/or of the alloy carbides may be greater than the melting point of the slag and of the inner part of the consumable electrode.

The outer part of the ingot may be hardened by a dispersion hardening effect of the alloy carbides.

Alternatively, the outer part of the rolled ingot may be hardened, additionally, or alternatively, by a secondary hardening heat treatment operation.

The electroslag remelting operation may be performed to provide a roll comprising an inner part having a first composition and a surface part having a second composition which is different from the first composition and the metal of the roll between the inner part and the surface part having a composition which changes from the first composition to the second composition without discontinuity. This may be achieved by inter-relating the voltage, and current and the slag composition of the electroslag remelting operation so that the molten bath is relatively flat.

Instead or in addition, the cooling rate of the mould may be adjusted as may be the rate of movement of the mould.

Alternatively, the electroslag remelting operation may he performed to provide a roll of substantially uniform composition throughout the cross-section of the roll.

By "electroslag remelting" (ESR) we mean a process in which a consumable electrode is melted beneath an electrical conductive slag in a moving mould from the lower end of which a continuously cast ingot emerges; the electrode is heated by thermal conduction from the slag and the slag is heated by electrical conduction from the electrode through the slag to a counter-electrode provided by the ingot.

In third and fourth alternatives, the roll may be a composite roll made by ESR cladding or spray cladding. In ESR cladding an arbor is clad using the electroslag re-melting method either utilising a wire feed as the stock material or a hollow electrode. In the former case, the coated particles may he introduced by a powder feed into the molten pool. In the latter case, either a powder feed may be used, or preferably, the coated particles may be incorporated into the hollow electrode during the primary melting and casting operation in a similar way to the production of the shell metal described above.

In spray cladding, the coated particles may be incorporated into a spray deposited layer. It is possible to produce a spray deposited layer hardened by the coated carbide particles of sufficient depth to provide the full working life of a rolling mill roll.

In a fifth alternative, a roll may be made by monobloc static casting where a roll is made simply by filling a stationary mould with a single engineering ferrous metal.

In a sixth alternative a roll may be made by a double poured static casting method wherein a roll is made by first partly filling a mould up to the top of a barrel part of the roll with an engineering ferrous metal of a desired composition for an outer shell part of the roll, made by the method of the first aspect of the invention or according to the second aspect of the invention which is provided with carbide particles, and, when an outer part of the shell metal has solidified, a metal of a desired core composition is fed into the bottom of the mould to dilute the first metal until a predetermined amount of metal has been displaced from an overflow between the ends and generally about halfway up, an upper journal part of the mould, the overflow is then closed and filling of the mould with the second metal is completed.

In a seventh alternative a roll is made by casting an ingot of metal made according to the first aspect of the invention or according to the second aspect of the invention and then forging the ingot to provide a forged roll followed by heat treating the forged roll.

A roll according to the present invention fulfils a market demand which has hitherto not been satisfactorily met by providing a roll having greater fracture toughness and spall resistance as well as having improved wear resistance.

A roll embodying the present invention is intended for use in the finishing stands of hot and cold strip mills. It may be used for roughing stands in hot strip mills and for other flat rolling purposes.

More particularly, a roll having said outer part made of the engineering ferrous metals listed below are intended for use in the respective applications specified.

| | |
|---|---|
| Indefinite Chill | All Stands Hot Strip |
| Chrome Iron | Early Stands Hot Strip |
| Chrome Iron | Cold Strip Mills |
| Alloy Steel | Hot Strip Mills |
| Tool Steel | Finishing Stands cold or hot Strip Mill |

The core may be flake, compact/vermicular or nodular cast iron, steel or other suitable material.

By providing particles which have an density which matches that of the engineering ferrous metal into which they are introduced segregation as a result of spin casting is avoided.

The spinning process tends to segregate less dense particles to the bore of the shell. Alloy carbide particles having a density which matches the parent metal results in the alloy carbide particles being distributed evenly throughout the section of the shell and not being centrifuged to the bore.

Engineering ferrous metals made by a method embodying the first aspect of the invention or according to the second aspect of the invention may be usefully used in other spin casting processes, for example, for producing liners for diesel engines and pipes such as for gas or oil, or other spin cast articles. Such as hollow sleeves for use in beam mills and other sections.

According to a fifth aspect of the invention, we provide a method of making a spun cast product wherein a metal made according to the first aspect of the invention or according to the second aspect of the invention is poured into a spin casting mould and a spin casting operation is performed thereon.

The invention, however, is not limited to products made by spin or centrifugal casting. The invention may be applied to a wide range of engineering ferrous metals for many purposes.

The engineering ferrous metals can be cast into conventional ingot moulds and subsequently forged into components, for example rolling mill rolls.

Rolls manufactured in this way would typically be hardened to a martensitic or bainite structure and would be used for the cold rolling of steel. For these applications a uniform structure is required to impart a uniform finish to the cold rolled product.

It is surprising that the carbide particles are distributed uniformly throughout the matrix and within the transformation carbide of the microstructure since it would be expected that on solidification the solidifying phase would push the alloy carbide particles in front of the solidifying liquid metal interface so that one would expect the alloy carbide particles to be segregated at the grain boundaries.

An example of the invention will now be described with reference to the accompanying drawings, wherein:
FIGURE 1 is a photomicrograph showing an inner region of a shell embodying the invention at a magnification of 500,
FIGURE 2 is an enlargement of part of Figure 1 at a magnification of 1,500,
FIGURES 3 and 4 are similar to Figures 2 and 3 but of a middle region of the shell,
FIGURES 5 and 6 are similar to Figures 1 and 2, but of an outer region of the shell,
FIGURE 7 is a photomicrograph of a shell of a roll of the same base composition but not embodying the invention at a magnification of x500,
FIGURE 8 is a photomicrograph of a forged test piece at a magnification of x400,
FIGURE 9 is a photomicrograph showing a sample of a second example of the invention at a magnification of x300,
FIGURE 10 is a scanning electron micrograph showing a sample of a third example of the invention at a magnification of x350,
FIGURE 11 is a scanning electron micrograph showing a sample of the third example of the invention at a magnification of x3000,
FIGURE 12 is a diagrammatic illustration of a spin casting plant used in Examples I - III,
FIGURE 13 is a diagrammatic side elevation of another embodiment showing an electroslag remelting apparatus when in use in a method embodying the present invention, and
FIGURE 14 is a transverse cross-section through a consumable electrode for use in the apparatus of Figure 13.

### EXAMPLE I

In a first example an engineering ferrous metal melt comprising an indefinite chill type iron having the following composition was made in conventional manner in an induction furnace.

| | |
|---|---|
| Carbon | 3.3% |
| Silicon | 0.85% |
| Manganese | 0.50% |
| Nickel | 2.3% |
| Chromium | 1.1% |
| Molybdenum | 0.1% |
| Sulfur | 0.050% |
| Phosphorus | 0.060% |
| Iron and usual incidentals | Balance |

After the iron had been brought to operating temperature, i.e, approximately 1500°C, a powder comprising alloy carbide particles surrounded by an iron coating with a carbon content of 3.00% were added to the melt in the melting furnace in an amount equivalent to 10% weight. The powder particles had a particle size of up to 500 microns and comprised:-

| | |
|---|---|
| 25% | Alpha Iron |
| 30% | Ti |
| 35% | W |
| Balance | C (of which 3% was free carbon) and usual incidentals. |

The alloy carbide particles had an average particle size of up to 10 microns and comprised a solid solution of 30% Ti and 35% W carbides and had a density of about 7 so as to match that of the iron.

The above mentioned operating temperature is higher than the usual temperature to which metal of the above composition is heated before tapping because the coating metal of the powder has a melting point of about 1520°C and it is desirable that the metal be as hot as possible. A temperature of higher than about 1500°C is not possible because of the tendency to "whiten" the indefinite chill iron.

The melt was then allowed to remain in the furnace for about 15 minutes to recover its operating temperature of approximately 1500°C. The molten metal was then poured into a ladle and then transferred in the ladle from the melting furnace to a conventional spin casting plant shown in Figure 1 where the metal was poured from the ladle into the spin casting plant to form a shell S of the above described metal in conventional manner. In order to make a composite rolling mill roll metal of suitable composition, such as nodular cast iron, would then be poured to form a core C. However, the present example was concerned with providing a shell, i.e. a tubular product, and so the core metal was not poured.

The dwell time of the metal in the furnace after adding the carbide particles was about 15 minutes to allow for temperature recovery and the dwell time in the ladle before pouring into the spin casting plant was about 15 minutes. Hence, in the present example about 30 minutes elapsed after adding the carbide particles and before casting. If desired the dwell time may be longer, e.g. 1 hour or 1.5 hours or more, or may be less.

After the shell had solidified samples were taken from regions adjacent the inner, middle and outer parts of the shell and suitable samples were prepared in conventional manner to obtain the photomicrographs shown in Figures 1 - 6.

It will be seen from these photomicrographs that the added carbide particles are distributed relatively uniformly on a macroscopic scale throughout the thickness of the shell. It is particularly to be noted that the carbide particles are not segregated at grain boundaries but are distributed relatively uniformly throughout the microstructure irrespective of the phases present as a result of phase transformation during solidification and cooling. It will be also seen from Figure 7 that the microstructure is of the same nature as in a comparison base material of the same composition but without alloy carbide particle addition.

A chemical analysis of a bulk sample was made which showed that only about half of the added carbide had been recovered to give 5 weight % of the carbide. By extra carbide we mean discrete carbide particles in addition to the carbide naturally present as a result of phase change on cooling.

From an Edax (energy dispersive X-ray) analysis, the ratio of Ti:W in the carbide was about 4:1, but this is on an atomic % basis, and on a corresponding Wt% basis, this gives
Ti:W as 1:1

The duplex nature of the carbides with a dark core suggests that the outer part of the carbide is W rich, and the inner Ti rich.

As mentioned above, the alloy carbide dispersion is uniform throughout the sample section and has an "area fraction" of about 5%, corresponding to a "volume fraction" of 5%. Whilst there is some evidence of clustering of the particles there are only a few particles in each cluster and the clustering is independent of the position of the particles in the engineering ferrous metal.

In particular there was no evidence that alloy carbide particles had been displaced ahead of the solidification interface, that is to say, the alloy carbide particle distribution was independent of the underlying microstructure.

The carbide particle size lay in the range 2 - 5 microns.

The hardness of the sample was tested and found to be VHN₃₀ 810 and the hardness of a sample cut from the comparison roll was found to be VHN₃₀ 650.

This increase in hardness of about 160 is somewhat greater than might be expected from the law of mixtures. It is believed that this is due to a small particle size hardening effect (Orowan hardening).

### EXAMPLE II

A composite roll comprising a shell made of Indefinite chill cast iron and a nodular cast iron core was made by a spin casting technique similar to that of Example I except that in this case a finished roll was made by pouring nodular cast iron core C after completion of the shell forming stage.

In this example the shell metal had the following composition:-

| | |
|---|---|
| T.C. - | 3.40 |
| Silicon - | 0.85 |
| Magnesium - | 0.51 |
| Nickel - | 4.13 |
| Chromium - | 1.63 |
| Molybdenum | 0.46 |
| Sulfur | 0.13 |
| Phosphorus | 0.35 |
| Copper | 0.06 |
| Lead | 0.0013 |
| Vanadium | 0.021 |
| Titanium | 0.175 |
| Iron and usual incidentals | Balance |

This metal was again made in an induction furnace and the metal in the induction furnace was heated above the melting point of the metal to the normal operating temperature, which, for example, is approximately 200°C above the liquidus temperature. In the present example the liquidus temperature was 1215°C and the operating temperature was 1460°C.

The induction furnace was provided with a cover and argon was fed into the interior of the cover but may be injected into the melt. The induction coil was turned off. The powder of coated alloy carbide particles was then injected into the melt by blowing through a lance with argon or in any other desired manner. If desired, instead of argon, any other inert gas may be used, or the closed space above the melt in the induction furnace may be connected to a vacuum and particles may be added in any desired manner, for example by gravity feed, particularly where the vacuum is provided. The induction coil was then turned on so that the melt was mixed. Other techniques to avoid oxidation may be used such as, use of a flux or addition of the coated alloy carbide powder as a cored wire, although the flux may inhibit dispersion of particles in the melt and a cored wire would be expensive.

The powder of coated alloy carbide particles comprises:-

| | |
|---|---|
| 27% | coating metal |
| 30% | Ti |
| 35% | W |
| Balance | C (of which 0.5% was free carbon) and usual incidentals. |

The coating metal comprised 59% Ni and 41% iron (including up to 0.5% free carbon and usual residuals).

After a suitable dwell time as mentioned above, the metal was poured into a ladle where it remained at a temperature corresponding to the liquidus temperature plus about 170 - 180°C and then the metal was cast into the mould of the spin casting plant wherein the temperature was the liquidus temperature plus about 80 - 110°C. The precise temperature depends upon the size, the smaller moulds being hotter and the larger cooler.

After the roll had solidified similar samples were taken as in Example I and Figure 9 is an optical D.I.C. (differential interference contrast) micrograph at x 300 magnification, unetched, of a sample taken from the middle of the shell and shows a matrix with graphite flakes and small uniformly and randomly distributed alloy carbide particles. The microstructure was similar to that of Example I with the alloy coated particles being distributed throughout the matrix and the transformation carbide.

A U.T.S. (ultimate tensile stress) test was performed on another sample from the shell and this showed the sample had a U.T.S. (Ultimate tensile stress) of 600 - 700 MPa. An indefinite chill cast iron of the same composition but without the alloy carbide particles has a U.T.S. (ultimate tensile stress) of 385-493 MPa.

### EXAMPLE III

A composite roll comprising a shell of High Chromium iron and a nodular cast iron core was made by the spin casting technique of Example II using an argon atmosphere.

The shell metal had the following composition:-

| | |
|---|---|
| T.C. | 2.95 |
| Si | 1.63 |
| S | 0.035 |
| P | 0.040 |
| Mn | 0.95 |
| Ni | 0.77 |
| Cr | 17.28 |
| Mo | 2.08 |
| Ca | 0.93 |
| Pb | 0.0081 |
| V | 0.031 |
| Fe and usual residuals | Balance |

The powder coated alloy carbide was as described in Example I. The powder was added to the metal in amounts equivalent to 10% by weight. 5% by weight was present in the solid metal.

The metal has a liquidus temperature of 1255°C and was heated to an operating temperature of 1560°C. The temperatures in the ladle and in the spin casting plant were related to the liquidus temperature similarly as in Example II the temperature on adding to the spin casting plant being 1345°C. After solidification of the roll samples were taken as in Example II.

Figure 10 is a scanning election microscope micrograph at x 350 magnification of a sample taken from the middle of the shell. Figure 11 is a similar micrograph but at x 3000 magnification. It will be seen that the discrete added alloy carbide particles are randomly and uniformly distributed and are present in both the matrix and in the transformation carbide. The carbide had largely separated into dark angular titanium rich particles about 1-10 micron in size and pinkish, rounded tungsten-rich particles generally less than about 5 micron in size. EDAX (energy dispersive X-ray) analysis revealed that the tungsten-rich particles also contains high levels of molybdenum whilst the metal itself contains low levels of titanium and tungsten in solution, both in the matrix and the transformation carbide. This points to the dissolution of the alloy carbide particles of (TiW)C in the melt, or at least their tungsten-rich outer layers, followed by their reprecipitation after solidification.

A U.T.S. (ultimate tensile stress) test was performed on a similar sample from the shell and this showed the sample had a U.T.S. (ultimate tensile stress) of 800-850 MPa. A high chromium iron of the same composition but without the alloy carbide addition has a U.T.S. (ultimate tensile stress) of 740-830 MPa.

### EXAMPLE IV

An engineering ferrous metal melt having the following composition was made in a conventional manner.

| T.C. | Si | Mn | Ni | Cr | Mo | Iron and usual incidentals |
|---|---|---|---|---|---|---|
| 0.8 | 0.28 | 0.35 | 0.5 | 2.0 | 0.25 | Balance |

After the steel had been brought to tapping temperature carbide particles of the same kind as described hereinbefore in connection with the first example were added to the melt in the melting furnace in an amount equivalent to 10% by weight.

The metal was then allowed to remain in the furnace as before to recover its tapping temperature and an ingot was then cast.

After the usual pouring section discard the ingot was 5½" in diameter and 6½" long and weighed 20kg.

This ingot was then step forged in an open die forge to form a round bar in three reductions as follows:
2:1 - 4½" diameter
4:1 - 3½" diameter
10:1 - 2" diameter

The resultant forging was heat treated to simulate a conventional forged roll heat treatment. Micrographs were taken at a magnification of x400 at different positions and on transverse and longitudinal sections. These showed that the forging had a substantially uniform microstructure throughout Figure 8 is an example of one of these micrographs taken on a longitudinal section.

It will be seen from these micrographs that the basic matrix structure was martensitic and that the added carbide particles again are distributed relatively uniformly throughout the forging. Again it was found that about half of the added carbide had been recovered to give 5% weight of the extra carbide.

### EXAMPLE V

Referring now to Figures 13 and 14, a further embodiment is illustrated. An electroslag remelting apparatus is shown in Figure 13 and is of essentially conventional kind comprising a cylindrical water cooled mould 10 which is movable vertically upwardly or downwardly. An electrode holder 11 holds, for example by being welded thereto, the upper end of a consumable electrode 12. Initially, the bottom end of the consumable electrode is immersed in molten slag 30 contained between a bottom plate 13 and the wall of the mould 10. Electric current is then passed to cause the lower end of the electrode to melt and as the droplets of metal fall from the lower end of the electrode 12 they pass through the slag and are refined and then solidify to form an ingot 14.

The basic operation of the electroslag remelting operation is entirely conventional as is the plant and hence further discussion is not necessary.

The consumable electrode 12 comprises an inner body 120 having welded to its external surface 121 a hollow cladding 122 which comprises a plurality of discrete tubular elements 123 in the form of tubes 124 containing powder 125.

The inner body 120 is made of low alloy steel, cast iron or mild steel such as 0.2% carbon steel.

The tubes 124 are made of mild steel in the present example but may be made of stainless steel and if desired the tubes may be made of high alloy steel or cast iron or indeed in any material of suitable composition such as

| | |
|---|---|
| Carbon | 0.5% - 3% |
| Aluminium | 0.0% - 1% |
| Molybdenum | 0.5% - 5% |
| Vanadium | 0.0% - 12% |
| Chromium | 0.5% - 15% |
| Tungsten | 0.0% - 8% |
| Silicon | 0.0% - 3% |
| Titanium | 0.0% - 8% |
| Nickel | 0.0% - 5% |
| Iron and usual residuals - | balance. |

Preferably, the tubes have a composition lying in the range:-

| | |
|---|---|
| Carbon | 0.5% - 3% |
| Aluminium | 0.0% - 0.1% |
| Molybdenum | 0.5% - 5.0% |
| Vanadium | 0.1% - 12% |
| Chromium | 0.5% - 15% |
| Tungsten | 0.1% - 8% |
| Silicon | 0.0% - 3% |
| Titanium | 0.1% - 8% |
| Nickel | 0.1% - 5% |
| Iron and usual residuals - | balance. |

The tube may have the following composition:

| | |
|---|---|
| Carbon | 1 % |
| Molybdenum | 2.5% |
| Vanadium | 0.7% |
| Chromium | 14% |
| Iron and usual residuals - | Balance |

The inner body may comprise a low alloy steel which may comprise:

| | |
|---|---|
| Carbon | 0.4% |
| Chromium | 1% |
| Nitrogen | up to 0.1% |
| Iron and usual residuals - | Balance |

If desired, the tubes may comprise other relatively high alloy metal such as:-

| | |
|---|---|
| Carbon | 3% |
| Molybdenum | 5% |
| Vanadium | 8% |
| Nickel | 2% |
| Iron and usual residuals - | balance |
| Carbon | 1% |
| Vanadium | 12% |
| Iron and usual residuals - | balance |
| Carbon | 2% |
| Tungsten | 5% |
| Titanium | 5% |
| Iron and usual residuals - | balance |
| Carbon | 3% |
| Silicon | 2% |
| Iron and usual residuals - | balance |

If desired, the inner body may comprise other relatively low alloy metal such as:-

| | |
|---|---|
| Carbon | 0.2% |
| Chromium | 0.5% |

or

| | |
|---|---|
| Carbon | 3% |
| Silicon | 2% |

or plain cast iron or mild steel.

However, the tubes may be provided solely to hold the powder 125 so could be composed of material of the same composition as the inner body or indeed may be made of suitable non-metallic material, such as silica, of a melting point so as to melt in the bath at a desired rate to release the alloying addition. The above described materials are applicable to hollow cladding of any suitable configuration.

In the present example the tubes have the following composition:

| | |
|---|---|
| Carbon | 0.2% |
| Iron and usual residuals - | balance |

The powder comprises a mixture of coated alloy carbide particles as described hereinbefore in connection with Example I (but may be any of the other coated alloy carbide particles described hereinbefore) and of particles of an alloying ingredient or ingredients.

For example, the powder may comprise:-

| | |
|---|---|
| Carbon | up to 10% (with 5% as graphite) |
| Tungsten | 35-40% |
| Titanium | 30-40% |
| Iron, carbide and usual residuals - | balance |

Some of the carbon is combined with the Tungsten and the Titanium as intermetallic compound but the Tungsten and Titanium are combined as a solid solution and a proportion of the Carbon present is as free graphite.

In the present example, the powder mixture has the following composition:

| | |
|---|---|
| Chromium | 2% |
| Tungsten | 40% |
| Titanium | 40% |
| Molybdenum | 1% |
| Vanadium | 1% |
| Carbon | 6% |
| Iron, carbide and usual residuals | Balance |

Alternatively, the powder mixture has the following composition:-

| | |
|---|---|
| Chromium | 2% |
| Tungsten | 35% |
| Titanium | 30% |
| Molybdenum | 1% |
| Vanadium | 1% |
| Carbon | 6% |
| Iron, carbide and usual residuals | Balance |

In general, one or more of the alloying elements may be present in the powder mixture, either as elements or combined with the carbon as inter-metallic compound or alloy.
Carbon
Molybdenum
Chromium
Tungsten
Titanium
Vanadium
Niobium

If desired the powder may be made of a powdered alloy of any one of the compositions or range of compositions described as being suitable for the tubes mentioned above or may be made of alloy of other compositions or of components which provide such compositions.

The amount of carbide particles added is such as to achieve up to 1-20% by volume of carbide particles in the surface part.

The tubes 124 in the present example are 16mm OD (outside diameter), 13mm ID (inside diameter) but may lie in the range from 6mm ID (inside diameter) to 28mm ID with appropriate (outside diameter) OD.

The tubes are provided with restrictions at intervals along their length so as to hold discrete amounts of carbide powder at positions along the length of the tubes, for example, such restrictions may be provided every 10cm.

In the present example the restrictions are provided by crimping the tubes so as to close or substantially to close their bore but, of course, such restrictions may be provided in any other desired way.

In the present example the tubes 124 are attached to the inner body 120 so as to extend longitudinally thereof parallel to the longitudinal axis of the inner body but, if desired, a single tube or tubes may be wound helically around the inner body or one or more tubes may extend circumferentially around the body so as to lie in a plane which is perpendicular to the longitudinal axis of the inner body so long as the tubes are of the correct size to hold the correct amount of powder to be released into the melt at the longitudinal position of the body.

Further alternatively, one or more tubes may be arranged to extend around the inner body in a plane or respective plane which is inclined to the longitudinal axis of the inner body at less than a right angle.

Although in this case cladding is in the form of discrete elements provided by the tubes 124 containing powder 125, if desired, the cladding may comprise a hollow sleeve, for example, a sleeve comprising inner and outer generally cylindrical walls inter-connected by generally annular shaped walls with the space between the walls containing powder as described hereinbefore and the sleeve being mounted, for example, by welding or by virtue of being a push fit on the inner body. In this case the hollow sleeve is provided with restrictions in its wall at suitable positions along the length of the sleeve so as to divide the powder into discrete amounts for release into the melt pool sequentially as the sleeve and inner body are melted.

In the present example the melting point of an alloy added with the carbides, for example Tungsten, Titanium solid solution, which can at least partly melt in the melt bath and of the alloy carbides are greater than the melting point of the slag 30 and of the inner body 120 of the consumable electrode 12. The melting point of the cladding tube/sleeve metal of the tubes and/or of any alloy ingredient may be 40"C below the melting point of the inner part 20 and 60°C above the melting point of the slag 30. The melting point of the tubes 22 is, in the present example, 1530°C.

The inner part may have a melting point lying in the range 1160"C to 1600°C and the cladding may have a melting point lying in the range 1160°C to 1600°C.

The melting point of the inner and outer parts may differ by 20°C to 60°C. The slag may have a melting point which differs from the lower of the melting point of the inner part and the cladding by 20°C to 60°C.

The mould is water cooled to a temperature lying in the range of 15°C to 65°C and the molten metal pool 31 has a temperature lying in the range 1400°C to 1600°C may be in the range 1160°C to 1600°C.

The voltage and current used in the electroslag remelting operation are manipulated so that there is a relatively high voltage and a relatively low current, or vice versa and in addition the composition of the slag is adjusted so as to provide a relatively viscous slag. As a result turbulence in the slag and the melt pool are minimised so that a desired composition gradient is achieved.

In addition, the voltage and current used are manipulated so that the floor of the melt pool is relatively flat.

The metal droplets leaving the cladding of the electrode, including the contents thereof, are more dense than the metal droplets leaving the inner body of the electrode when they are more highly alloyed. This results in the droplets from the cladding of the electrode falling downwardly adjacent to the wall of the mould and, because the floor of the melt pool is relatively flat, there is relatively little tendency for these droplets to run towards the middle of the melt pool before they have solidified as a result of their spatial and temperature proximity to the mould wall.

The composition of the slag is adjusted to reduce the ionic capacity of the slag by adjusting the balance of the silicon, calcium and aluminium in the slag to reduce the tendency for electromagnetic stirring as well as the composition of the slag being adjusted to provide a relatively higher viscosity.

Typically the slag has the following composition:- 33¹/₃% CaO, 33¹/₃% CaF₂, 33¹/₃% Al₂0₃.

However the slag may have a composition of 20% CaO, 80% CaF₂, 0% Al₂0₃.

The cooling rate provided by the water cooling to the mould may be adjusted by adjusting the raw temperature of the mould to lie in the range 15°C to 65°C. In addition, the rate of movement of the mould may also be adjusted.

Typically, the electrode has a diameter which is about 0.9% of the diameter of the mould cavity.

The electrode is arranged so that approximately 20%, by weight, of the electrode comprises cladding and the balance is provided by the inner body. This ratio may lie in the range 1% to 40%.

Although above the melting point of the cladding has been described as being lower than the melting point of the metal of the inner body, if desired this may be reversed.

As the electrode 12 melts, droplets of liquid metal are solid particles of the metal carbide which does not melt, from the tubes 124 and powder 125 fall generally vertically downwardly and because of the relatively close spatial and temperature proximity to the wall of the mould 110 the droplets solidify relatively rapidly, at or adjacent to the mould wall and the carbide particles are trapped by the solidifying melt adjacent the mould wall, so that the metal at the surface of the ingot 14 has a relatively high uniform distribution of alloy and alloy carbides as well as having a composition of matrix substantially similar to the composition of the metal of the tubes 124.

The metal droplets falling from the middle of the bottom of the inner part fall vertically downwardly and thus the metal solidifying at the centre of the ingot has a composition substantially similar to the composition of the inner part of the electrode.

This is facilitated where metal from the cladding is of greater density than the metal from the inner body as this causes the droplets to fall downwardly adjacent to the mould wall together and by the hereinbefore mentioned precautions to avoid mixing, low slag viscosity, low slag electromagnetic stirring and a relatively flat melt pool base.

Between these two extremes there is limited mixing of the material from the two regions so that a change in composition between the two extremes takes place without discontinuity. Accordingly, the ingot has a relatively uniform transition region between the inner part and the surface part. The ingot, and hence any resulting product such as a roll as described hereinbefore, has an elastic modulus which increases in direct proportion to the amount of the distribution of the alloy/alloy carbide through the ingot cross-section.

In the present example the composition at the surface of the ingot is:

| | |
|---|---|
| Carbon | 0.5% |
| Molybdenum | 0.2% |
| Vanadium | 0.9% |
| Tungsten | 1.2% |
| Chromium | 0.5% |
| Titanium | 0.15% |
| Iron, carbide and usual residuals | balance |

The composition at the centre of the ingot is:

| | |
|---|---|
| Carbon | 0.5% |
| Molybdenum | 0.1% |
| Tungsten | 0.3% |
| Titanium | 0.03% |
| Vanadium | 0.2% |
| Chromium | 0.5% |
| Iron, carbide and usual residuals | balance |

The variation in composition is believed to arise due to the relatively higher diffusion of chromium and carbon compared with the relatively lower diffusion and more dense tungsten and titanium.

The composition gradient does not exceed 40% per 100mm in the radial direction and this condition applies with any position along the longitudinal extent of the roll.

### EXAMPLE VI

In this example, the electroslag remelting apparatus and method of operation described in connection with Example V may also used but with the operating conditions modified so as to aim to provide a uniform composition roll, for example the voltage and current used manipulated so that the floor of the melt pool is relatively deep. Generally, conventional operating conditions and slag compossations were used.

An electrode comprising an inner part, with an outer cladding of tubular configuration both made of low carbon steel was made with the space therebetween containing alloy carbide powder as described in connection with Example V. Quantities were calculated for a target addition of 1 wt%.

A conventional electroslag remelting operation was performed.

Hardness tests were performed on the remelting roll and this revealed that throughout the majority of the cross-section of the roll a hardness of around Hv 250 was achieved.

This is considerably above that expected according to the law of mixtures where for a 1% addition of carbide (Hv approximately 3000) to a low carbon steel (Hv approximately 180) a value of around Hv 210 is expected.

Examination of the microstructure revealed a good uniform and random dispersion of added carbide particles with a volume approaching 1% by weight.

EDAX (energy dispersive X-ray) analysis of individual carbide particles shows a strong presence of titanium with only traces of tungsten. This suggests that solution of tungsten from the particles has occurred in the melt. This would retard the pearlite transformation cooling allowing a bainitic structure to develop and thus giving a greater hardness due to the modification of phase transformations in this way.

Moreover, since the low carbon steel of this example contained about 0.1% nitrogen it is considered that at least some of this nitrogen has formed titanium carbo-nitride particles and hence that at least some of the above mentioned carbide particles comprise such titanium carbo-nitride particles which may also contain tungsten.

Unless otherwise stated compositions are expressed herein in % by weight.

References to particle size are to the largest dimension of the largest particle unless otherwise described.

## Claims (Claims for the following Contracting State(s): BE, DE, ES, FR, GB, IT, LU, NL, SE)

1. A method of making a rolling mill roll comprising the steps of adding to liquid cast iron or steel, solid alloy carbide particles and thereafter permitting the cast iron or steel to solidify wherein the alloy carbide particles have a density of 6 to 8 g per cm³ which matches that of the cast iron or steel, and the solid carbide particles are coated with a metal which allows wetting to occur between the particles and the liquid cast iron or steel and casting said metal to provide at least an outer part of said roll.

2. A method according to claim 1 wherein the coating metal comprises iron or an iron carbon alloy, or an alloy of two or more elements selected from the group comprising iron, nickel, copper, titanium and carbon, or nickel or copper and usual incidentals, and/or nitrogen.

3. A method according to claim 1 or 2 wherein the coating metal has a melting point which is within approximately 20°-30°C of the temperature of the engineering ferrous metal at which said coated carbide particles are added.

4. A method according to any one of the preceding claims wherein the alloy carbide particles are coated with iron or with an iron alloy having a lower carbon content than that of the cast iron or steel to which they are added and the coated alloy carbide particles are added to the cast iron or steel and permitted to dwell therein sufficiently long for carbon from the cast iron or steel to diffuse into the coating and so produce a composition which has a melting point which matches the operating temperature of the cast iron or steel.

5. A method according to any one of the preceding claims wherein the coated alloy carbide particles are added to the liquid cast iron or steel either in the melting furnace or in a ladle into which the metal has been poured from the melting furnace, or in the stream of metal being poured from the melting furnace to the ladle, or in the stream of metal being poured from the ladle into a mould.

6. A method according to claim 5 wherein the coated alloy carbide particles are added in the melting furnace.

7. A method according to any one of the preceding claims wherein the coated alloy carbide particles are added to the cast iron or steel in an inert environment.

8. A method according to any one of the preceding claims wherein the coated alloy carbide particles are added to the cast iron or steel melt in the form of a powder comprising powder particles having a particle size up to 2mm and preferably of about 500 micro-meters (500 microns) and containing alloy carbide particles having a particle size of up to 10 micro-meters (10 microns) and preferably in the range 1-5 micro-meters (1.5 microns) and more preferably 2.5 micro meters (2-5 microns).

9. A method according to any one of the preceding claims wherein the coated alloy carbide particles are added to the cast iron or steel melt in the form of a powder wherein the powder particles comprise:-
| | |
|---|---|
| 25% | coating metal |
| 30% | Ti |
| 35% | W |
| Balance | C (of which 3.5% was free carbon) and usual incidentals. |

10. A method according to any one of the preceding claims wherein the coating metal comprises wholly or substantially wholly alpha iron and up to 3.5% free carbon.

11. A method according to any one of Claims 1 to 8 wherein the coated alloy carbide particles are added to the cast iron or steel melt in the form of a powder wherein the powder particles comprise:-
| | |
|---|---|
| 27% | coating metal |
| 30% | Ti |
| 35% | W |
| Balance | C (of which 0.5% was free carbon) and usual incidentals. |

12. A method according to any one of Claims 1 to 8 or claim 11 wherein the coating metal comprises an alloy of iron, nickel and carbon.

13. A method according to Claim 12 wherein the alloy of iron, nickel and carbon comprises:-
| | |
|---|---|
| 59% | nickel |
| 41% | iron and up to 0.5% free carbon and usual incidentals. |

14. A method according to any one of Claims 1 to 4 or any one of Claims 8 to 13 when dependant on any one of Claims 1 to 4 wherein the coated alloy carbide particles are added during an electroslag remelting operation.

15. A method according to any one of the preceding claims wherein the alloy carbide is selected from the group comprising chromium, molybdenum, titanium, tungsten, niobium, vanadium or nixed carbides thereof such as Cr₇C₃, (CrMo)₇C₃ or mixed carbo-nitrides thereof.

16. A method according to any one of the preceding claims wherein the carbide is a mixed tungsten titanium carbide of the kind (TiW)C where the ratio of titanium to tungsten is about 1:1 by weight and preferably in the ratio range:
1:1 to 1:1.1

17. A method according to any one of the preceding claims wherein the alloy carbide particles have a maximum dimension of up to 10 micro-meters (10 microns) and preferably 1-5 micro-meters (1 - 5 microns) and more preferably 2-5micro-meters (2-5 microns).

18. A method according to any one of the preceding claims wherein the amount of alloy carbide particles added is such as to achieve up to 20%, preferably up to 5 to 20%, by volume of alloy carbide particles in the solid metal.

19. A method according to claim 18 wherein the alloy carbide content is in the range 0.1 to 20% by volume and more preferably 3 to 10% when a hardening effect based on the law of mixtures is provided.

20. A method according to claim 18 wherein the alloy carbide content is in the range from 1% to about 0.5% by volume or from 1% to about 0.1% by volume or less when a hardening effect based on a modification of the transformation of the microstructure is provided.

21. A method according to any one of the preceding claims wherein the cast iron or steel is selected from the group comprising iron, chromium iron, high alloy steel, tool steel, medium alloy steel, low alloy steel, S.G. iron, steel or cast iron having a carbon content lying in the range 0.3- 3.8% and which may contain nitrogen up to 0.1%.

22. A rolling mill roll having at least an outer part which comprises a cast iron or steel product comprising a carbon alloy having a micro-structure which has resulted from phase transformation on cooling and having dispersed therein discrete alloy carbide particles wherein the alloy carbide has a composition so that the density of the alloy carbide lying in the range of 6 to 8 g per cm³ matches that of the cast iron or steel.

23. A rolling mill roll according to Claim 22 wherein the microstructure comprises a matrix and transformation carbide which have resulted from phase transformation of the engineering ferrous metal.

24. A rolling mill roll according to Claim 23 wherein the discrete alloy carbide particles are distributed in the matrix.

25. A rolling mill roll according to Claim 23 or claim 24 wherein the discrete alloy carbide particles are distributed in the transformation carbide.

26. A rolling mill roll according to any one of Claims 22 to 25 wherein the discrete alloy carbide particles are uniformly distributed in the microstructure.

27. A rolling mill roll according to any one of the preceding claims wherein the alloy carbide is selected from the group comprising chromium,, molybdenum, titanium, tungsten, niobium, vanadium or mixed carbides thereof such as Cr₇C₃, (CrMo)₇C₃ or mixed carbo-nitrides thereof.

28. A rolling mill roll according to any one of the preceding claims wherein the carbide is a mixed tungsten titanium carbide of the kind (TiW)C where the ratio of titanium to tungsten is about 1:1 by weight and preferably in the ratio range:
1:1 to 1:1.17

29. A rolling mill roll according to any one of the preceding claims wherein the alloy carbide particles have a maximum dimension of up to 10 micro-meters (10 microns) and preferably 1-5 micro-meters (1-5 microns) and more preferably 2-Smicro-meters (2-5 microns).

30. A rolling mill roll according to any one of the preceding claims wherein the amount of alloy carbide particles added is such as to achieve up to 20%, preferably upto 5 to 20%, by volume of alloy carbide particles in the solid metal.

31. A rolling mill roll according to Claim 30 wherein the alloy carbide content is in the range 0.1 to 20% by volume and more preferably 3 to 10% when a hardening effect based on the law of mixtures is provided.

32. A rolling mill roll according to Claim 30 wherein the alloy carbide content is in the range from 1% to about 0.5% by volume or from 1% to about 0.1% by volume or less when a hardening effect based on a modification of the transformation of the microstructure is provided.

33. A rolling mill roll according to any one of the preceding claims wherein the cast iron or steel is selected from the group comprising iron, chromium iron, high alloy steel, tool steel, medium alloy steel, low alloy steel, S.G. iron, steel or cast iron having a carbon content lying in the range 0.3 - 3.8% and which may contain nitrogen up to 0.1%.

34. A method according to any one of claims 1 to 21 wherein the rolling mill roll is a composite rolling mill roll of the kind having a core and an outer shell with, optionally, at least one intermediate layer, in which the shell comprises said outer part.

35. A rolling mill roll according to any none of claims 22 to 33 wherein the rolling mill roll is a composite rolling mill roll of the kind having a core and an outer shell with, optionally, at least one intermediate layer, in which the shell comprises said outer part.

36. A method according to Claim 34 wherein the alloy carbide particles are introduced into a molten engineering ferrous metal of which the shell is to be formed and then the engineering ferrous metal with the alloy carbide particles therein is poured into a mould.

37. A method according to Claim 34 or Claim 36 wherein the composite roll is made by centrifugal casting.

38. A method according to any one of Claims 1 to 21 wherein the roll is made by performing an electroslag remelting operation on a consumable electrode which comprises an inner body provided with an external cladding comprising a hollow element containing said coated alloy carbide particles.

39. A method according to Claim 38 wherein the hollow element also contains a powder alloy ingredient.

40. A method according to Claim 38 or Claim 39 wherein the electroslag remelting operation is performed to provide a roll comprising an inner part having a first composition and a surface part having a second composition which is different from the first composition and the metal of the roll between the inner part and the surface part having a composition which changes from the first composition to the second composition without discontinuity.

41. A method according to Claim 38 or claim 40 wherein the electroslag remelting operation is performed to provide a roll of substantially uniform composition throughout the cross-section of the roll.

42. A method according to Claim 34 or claim 36 wherein the roll is made by electroslag remelting cladding or spray cladding.

43. A method according to any one of claims 1 to 21 wherein the roll is made by monobloc static casting by filling a stationary mould with a single cast iron or steel.

44. A method according to any one of claims 1 to 21 wherein a roll is made by a double poured static casting method.

45. A method according to any one of Claims 34, 36, 37 to 39 or claims 42 to 44 wherein the core comprises flake, compact, vermicular or nodular cast iron, or steel.

46. A method according to any one of Claims 1 to 21 comprising casting an ingot of said metal and then forging the ingot to provide a forged roll followed by heat treating the forged roll.

47. A rolling mill roll according to any one of claims 22 to 33, or 35 wherein the rolling mill roll is a forged roll.

## Claims (Claims for the following Contracting State(s): AT, CH LI , DK, GR, IE, MC, PT)

1. A method of making cast iron or steel comprising the steps of adding to cast iron or steel, solid alloy carbide particles and thereafter permitting the cast iron or steel to solidify wherein the alloy carbide particles have a density lying in the range 6-8 g per cm³ to match that of the cast iron or steel and wherein the solid carbide particles arc coated with a metal which allows wetting to occur between the particles and the liquid cast iron or steel metal.

2. A method according to claim 1 wherein the coating metal comprises iron or an iron carbon alloy, or an alloy of two or more elements selected from the group comprising iron, nickel, copper, titanium and carbon, or nickel or copper and usual incidentals, and/or nitrogen.

3. A method according to claim 1 or 2 wherein the coating metal has a melting point which is within approximately 20°-30°C of the temperature of the cast iron or steel at which said coated carbide particles are added.

4. A method according to any one of the preceding claims wherein the alloy carbide particles are coated with iron or with an iron alloy having a lower carbon content than that of the cast iron or steel to which they are added and the coated alloy carbide particles are added to the cast iron or steel and permitted to dwell therein sufficiently long for carbon from the cast iron or steel to diffuse into the coating and so produce a composition which has a melting point which matches the operating temperature of the cast iron or steel.

5. A method according to any one of the preceding claims wherein the coated alloy carbide particles are added to the liquid cast iron or steel either in the melting furnace or in a ladle into which the metal has been poured from the melting furnace, or in the stream of metal being poured from the melting furnace to the ladle, or in the stream of metal being poured from the ladle into a mould.

6. A method according to claim 5 wherein the coated alloy carbide particles are added in the melting furnace and wherein the melting furnace is an induction furnace.

7. A method according to any one of the preceding claims wherein the coated alloy carbide particles are added to the cast iron or steel in an inert environment.

8. A method according to any one of the preceding claims wherein the coated alloy carbide particles are added to the cast iron or steel melt in the form of a powder comprising powder particles having a particle size up to 2mm and preferably of about 500 micro-meters (500 microns) and containing alloy carbide particles having a particle size of up to 10 micro-meters (10 microns) and preferably in the range 1-5 micro-meters (1.5 microns) and more preferably 2.5 micro meters (2-5 microns).

9. A method according to any one of the preceding claims wherein the coated alloy carbide particles are added to the cast iron or steel melt in the form of a powder wherein the powder particles comprise:-
| | |
|---|---|
| 25% | coating metal. |
| 30% | Ti |
| 35% | W |
| Balance | Carbon (including up to 3.5% free carbon) and usual incidentals. |

10. A method according to any one of the preceding claims wherein the coating metal comprises wholly or substantially wholly alpha iron and up to 3.5% free carbon.

11. A method according to any one of Claims 1 to 8 wherein the coated alloy carbide particles are added to the cast iron or steel melt in the form of a powder wherein the powder particles comprise:-
| | |
|---|---|
| 27% | coating metal. |
| 30% | Ti |
| 35% | W |
| Balance | Carbon (including up to 0.5% free carbon) and usual incidentals. |

12. A method according to any one of Claims 1 to 8 or claim 11 wherein the coating metal comprises an alloy of iron, nickel and carbon.

13. A method according to Claim 12 wherein the alloy of iron, nickel and carbon comprises:-
| | |
|---|---|
| 59% | nickel |
| 41% | iron and up to 0.5% free carbon and usual incidentals. |

14. A method according to any one of Claims 1 to 4 or any one of Claims 8 to 13 when dependant on any one of Claims 1 to 4 wherein the coated alloy carbide particles are added during an electroslag remelting operation.

15. A method according to any one of the preceding claims wherein the alloy carbide is selected from the group comprising chromium, molybdenum, titanium, tungsten, niobium, vanadium or mixed carbides thereof such as Cr₇C₃, (CrMo)₇C₃ or mixed carbo-nitrides thereof.

16. A method according to any one of the preceding claims wherein the carbide is a mixed tungsten titanium carbide of the kind (TiW)C where the ratio of titanium to tungsten is about 1:1 by weight and preferably in the ratio range:
1:1 to 1:1.17

17. A method according to any one of the preceding claims wherein the alloy carbide particles have a maximum dimension of up to 10 micro-meters (10 microns) and preferably 1-5 micro-meters (1 - 5 microns) and more preferably 2-5micro-meters (2-5 microns).

18. A method according to any one of the preceding claims wherein the amount of alloy carbide particles added is such as to achieve up to 20%, preferably up to 5 to 20%, by volume of alloy carbide particles in the solid metal.

19. A method according to claim 18 wherein the alloy carbide content is in the range 0.1 to 20% by volume and more preferably 3 to 10% when a hardening effect based on the law of mixtures is provided.

20. A method according to claim 18 wherein the alloy carbide content is in the range from 1% to about 0.5% by volume or from 1% to about 0.1% by volume or less when a hardening effect based on a modification of the transformation of the microstructure is provided.

21. A method according to any one of the preceding claims wherein the cast iron or steel is selected from the group comprising iron, chromium iron, high alloy steel, tool steel, medium alloy steel, low alloy steel, S.G. iron, steel or cast iron having a carbon content lying in the range 0.3 - 3.8% and which may contain nitrogen up to 0.1%.

22. An cast iron or steel product comprising an iron carbon alloy having a micro-structure which has resulted from phase transformation on cooling and having dispersed therein discrete alloy carbide particles wherein the alloy carbide has a composition so that the density of the alloy carbide lying in the range of 6-8 g per cm³ matches that of the cast iron or steel.

23. A product according to Claim 22 wherein the microstructure comprises a matrix and transformation carbide which have resulted from phase transformation of the cast iron or steel.

24. A product according to Claim 23 wherein the discrete alloy carbide particles are distributed in the matrix.

25. A product according to Claim 23 or claim 24 wherein the discrete alloy carbide particles are distributed in the transformation carbide.

26. A product according to any one of Claims 22 to 25 wherein the discrete alloy carbide particles are uniformly distributed in the microstructure.

27. A product according to any one of the preceding claims wherein the alloy carbide is selected from the group comprising chromium, molybdenum, titanium, tungsten, niobium, vanadium or mixed carbides thereof such as Cr₇C₃, (CrMo)₇C₃ or mixed carbo-nitrides thereof.

28. A product according to any one of the preceding claims wherein the carbide is a mixed tungsten titanium carbide of the kind (TiW)C where the ratio of titanium to tungsten is about 1:1 by weight and preferably in the ratio range:
1:1 to 1:1.17

29. A product according to any one of the preceding claims wherein the alloy carbide particles have a maximum dimension of up to 10 micro-meters (10 microns) and preferably 1-5 micro-meters (1-5 microns) and more preferably 2-5micro-meters (2-5 microns).

30. A product according to any one of the preceding claims wherein the amount of alloy carbide particles added is such as to achieve up to 20%, preferably upto 5 to 20%, by volume of alloy carbide particles in the solid metal.

31. A product according to Claim 30 wherein the alloy carbide content is in the range 0.1 to 20% by volume and more preferably 3 to 10% when a hardening effect based on the law of mixtures is provided.

32. A product according to Claim 30 wherein the alloy carbide content is in the range from 1% to about 0.5% by volume or from 1% to about 0.1% by volume or less when a hardening effect based on a modification of the transformation of the microstructure is provided.

33. A product according to any one of the preceding claims wherein the cast iron or steel is selected from the group comprising iron, chromium iron, high alloy steel, tool steel, medium alloy steel, low alloy steel, S.G. iron, steel or cast iron having a carbon content lying in the range 0.3 - 3.8% and which may contain nitrogen up to 0.1%.

34. A method of making a rolling mill roll wherein a metal made according to any one of Claims 1 to 21 or a metal according to any one of Claims 22 to 33 is cast to make at least an outer part of the rolling mill roll.

35. A method according to Claim 34 wherein the rolling mill roll is a composite rolling mill roll of the kind having a core and an outer shell with, optionally, at least one intermediate layer, in which the shell comprises said outer part.

36. A product according to any one of claims 15 to 19 or claims 22 to 33 wherein the product is a rolling mill roll.

37. A product according to claim 36 wherein the rolling mill roll is a composite rolling mill roll of the kind having a core and an outer shell with, optionally, at least one intermediate layer, in which the shell comprises said outer part.

38. A method according to Claim 35 wherein the alloy carbide particles are introduced into a molten cast iron or steel of which the shell is to be formed and then the cast iron or steel with the alloy carbide particles therein is poured into a mould.

39. A method according to Claim 35 or Claim 38 wherein the composite roll is made by centrifugal casting.

40. A method according to any one of Claims 1 to 21 wherein the roll is made by performing an electroslag remelting operation on a consumable electrode which comprises an inner body provided with an external cladding comprising a hollow element containing said coated alloy carbide particles.

41. A method according to Claim 40 wherein the hollow element also contains a powder alloy ingredient.

42. A method according to Claim 40 or Claim 41 wherein the electroslag remelting operation is performed to provide a roll comprising an inner part having a first composition and a surface part having a second composition which is different from the first composition and the metal of the roll between the inner part and the surface part having a composition which changes from the first composition to the second composition without discontinuity.

43. A method according to Claim 40 or claim 42 wherein the electroslag remelting operation is performed to provide a roll of substantially uniform composition throughout the cross-section of the roll.

44. A method according to Claim 34 or a claim 35 wherein the roll is made by electroslag remelting cladding or spray cladding.

45. A method according to any one of claims 1 to 14 or claims 20 to 26 when dependent on any one of claims 1 to 14 wherein the roll is made by monobloc static casting by filling a stationary mould with a single cast iron or steel.

46. A method according to any one of claims 1 to 21 wherein a roll is made by a double poured static casting method.

47. A method according to any one of Claims 34, 35, 38 to 41 or claims 44 to 46 wherein the core comprises flake, compact, vermicular or nodular cast iron, or steel.

48. A method according to any one of Claims 1 to 21 comprising casting an ingot of said metal and then forging the ingot to provide a forged roll followed by heat treating the forged roll.

49. A product according to claim 36 wherein the rolling mill roll is a forged roll.

50. A method according to any one of Claims 1 to 21 when said cast iron or steel is poured into a centrifugal casting mould and a centrifugal casting operation is performed thereon to provide a centrifugal cast product.

51. A product according to any one of claims 22 to 33 wherein the product is a centrifugally cast product.

## Patentansprüche (Patentansprüche für folgende(n) Vertragsstaat(en): BE, DE, ES, FR, GB, IT, LU, NL, SE)

1. Verfahren zur Herstellung einer Walzwerkwalze, welches die Schritte umfaßt, daß zu flüssigem Gußeisen oder Stahl feste Legierungscarbidteilchen zugegeben werden und man danach das Gußeisen oder den Stahl fest werden läßt, wobei die Legierungcarbidteilchen eine Dichte von 6 bis 8 g pro cm³ aufweisen, die mit derjenigen des Gußeisens oder Stahls zusammenpaßt, und die festen Carbidteilchen mit einem Metall beschichtet sind, das zuläßt, daß Benetzung zwischen den Teilchen und dem flüssigen Gußeisen oder Stahl auftritt, und daß besagtes Metall gegossen wird, um wenigstens einen äußeren Teil besagter Walze bereitzustellen.

2. Verfahren nach Anspruch 1, dadurch gekennzeichnet, daß das Beschichtungsmetall Eisen umfaßt oder eine Eisen-Kohlenstoff-Legierung oder eine Legierung aus zwei oder mehr Elementen, die ausgewählt sind aus der Gruppe, die Eisen, Nickel, Kupfer, Titan und Kohlenstoff umfaßt, oder Nickel oder Kupfer und übliche Nebenbestandteile, und/oder Stickstoff.

3. Verfahren nach Anspruch 1 oder 2, dadurch gekennzeichnet, daß das Beschichtungsmetall einen Schmelzpunkt besitzt, der innerhalb von ungefähr 20°-30°C der Temperatur des technischen Eisenmetalls liegt, bei der besagte beschichtete Carbidteilchen zugegeben werden.

4. Verfahren nach einem der vorangehenden Ansprüche, dadurch gekennzeichnet, daß die Legierungscarbidteilchen mit Eisen oder mit einer Eisenlegierung, die einen niedrigeren Kohlenstoffgehalt aufweist als derjenige des Gußeisens oder Stahls, zu dem sie zugegeben werden, beschichtet werden und die beschichteten Legierungscarbidteilchen zum Gußeisen oder Stahl zugegeben und darin ausreichend lange belassen werden, damit Kohlenstoff aus dem Gußeisen oder Stahl in die Beschichtung hinein diffundiert und so eine Zusammensetzung erzeugt, die einen Schmelzpunkt hat, der mit der Betriebstemperatur des Gußeisens oder Stahls zusammenpaßt.

5. Verfahren nach einem der vorangehenden Ansprüche, dadurch gekennzeichnet, daß die beschichteten Legierungscarbidteilchen zum flüssigen Gußeisen oder Stahl entweder im Schmelzofen oder in einer Pfanne, in die das Metall aus dem Schmelzofen gegossen worden ist, oder im Metallstrom, der aus dem Schmelzofen in die Pfanne gegossen wird, oder im Metallstrom, der aus der Pfanne in eine Form gegossen wird, zugegeben werden.

6. Verfahren nach Anspruch 5, dadurch gekennzeichnet, daß die beschichteten Legierungscarbidteilchen im Schmelzofen zugegeben werden.

7. Verfahren nach einem der vorangehenden Ansprüche, dadurch gekennzeichnet, daß die beschichteten Legierungscarbidteilchen zum Gußeisen oder Stahl in einer inerten Umgebung zugegeben werden.

8. Verfahren nach einem der vorangehenden Ansprüche, dadurch gekennzeichnet, daß die beschichteten Legierungscarbidteilchen zur Gußeisen- oder Stahlschmelze in der Form eines Pulvers zugegeben werden, das Pulverteilchen mit einer Teilchengröße von bis zu 2 mm und vorzugsweise etwa 500 Mikrometern (500 Mikrons) umfaßt und Legierungscarbidteilchen mit einer Teilchengröße von bis zu 10 Mikrometern (10 Mikrons) und vorzugsweise im Bereich 1-5 Mikrometer (1,5 Mikrons) und bevorzugter 2,5 Mikrometer (2-5 Mikrons) enthält.

9. Verfahren nach einem der vorangehenden Ansprüche, dadurch gekennzeichnet, daß die beschichteten Legierungscarbidteilchen zur Gußeisen- oder Stahlschmelze in der Form eines Pulvers zugegeben werden, wobei die Pulverteilchen umfassen:
| | |
|---|---|
| 25% | Beschichtungsmetall |
| 30% | Ti |
| 35% | W |
| Rest | Kohlenstoff (einschließlich bis zu 3,5 % freier Kohlenstoff) und übliche Nebenbestandteile |

10. Verfahren nach einem der vorangehenden Ansprüche, dadurch gekennzeichnet, daß das Beschichtungsmetall vollständig oder im wesentlichen vollständig Alpha-Eisen und bis zu 3,5 % freien Kohlenstoff umfaßt.

11. Verfahren nach einem der Ansprüche 1 bis 8, dadurch gekennzeichnet, daß die beschichteten Legierungscarbidteilchen zur Gußeisen- oder Stahlschmelze in der Form eines Pulvers zugegeben werden, wobei die Pulverteilchen umfassen:
| | |
|---|---|
| 27% | Beschichtungsmetall |
| 30% | Ti |
| 35% | W |
| Rest | Kohlenstoff (einschließlich bis zu 0,5 % freier Kohlenstoff) und übliche Nebenbestandteile |

12. Verfahren nach einem der Ansprüche 1 bis 8 oder Anspruch 11, dadurch gekennzeichnet, daß das Beschichtungsmetall eine Legierung aus Eisen, Nickel und Kohlenstoff umfaßt.

13. Verfahren nach Anspruch 12, dadurch gekennzeichnet, daß die Legierung aus Eisen, Nickel und Kohlenstoff umfaßt:
| | |
|---|---|
| 59% | Nickel |
| 41% | Eisen und bis zu 0,5 % freien Kohlenstoff und übliche Nebenbestandteile |

14. Verfahren nach einem der Ansprüche 1 bis 4 oder einem der Ansprüche 8 bis 13, sofern abhängig von einem der Ansprüche 1 bis 4, dadurch gekennzeichnet, daß die beschichteten Legierungscarbidteilchen während eines Elektroschlacke-Umschmelzprozesses zugegeben werden.

15. Verfahren nach einem der vorangehenden Ansprüche, dadurch gekennzeichnet, daß das Legierungscarbid ausgewählt ist aus der Gruppe, die aus Chrom-, Molybdän-, Titan-, Wolfram-, Niob-, Vanadium- oder Mischcarbiden derselben besteht, wie etwa Cr₇C₃, (CrMo)₇C₃ oder gemischten Carbonitriden derselben.

16. Verfahren nach einem der vorangehenden Ansprüche, dadurch gekennzeichnet, daß das Carbid ein gemischtes wolfiam-Titan-Carbid der Art (TiW)C ist, wobei das Gewichtsverhältnis von Titan zu Wolfram etwa 1:1 beträgt und vorzugsweise im Verhältnisbereich liegt:
1:1 bis 1:1.17

17. Verfahren nach einem der vorangehenden Ansprüche, dadurch gekennzeichnet, daß die Legierungscarbidteilchen eine maximale Abmessung von bis zu 10 Mikrometern (10 Mikrons) und vorzugsweise 1-5 Mikrometer (1-5 Mikrons) und bevorzugter 2-5 Mikrometer (2-5 Mikrons) besitzen.

18. Verfahren nach einem der vorangehenden Ansprüche, dadurch gekennzeichnet, daß die zugegebene Menge an Legierungscarbidteilchen derart ist, daß bis zu 20 %, vorzugsweise bis zu 5 bis 20 %, volumenbezogen, Legierungscarbidteilchen im festen Metall erreicht werden.

19. Verfahren nach Anspruch 18, dadurch gekennzeichnet, daß der Legierungscarbidgehalt im Bereich 0,1 bis 20 Vol.-% und bevorzugter 3 bis 10 % liegt, wenn eine Härtungswirkung auf der Basis des Gesetzes der Mischungen bereitgestellt wird.

20. Verfahren nach Anspruch 18, dadurch gekennzeichnet, daß der Legierungscarbidgehalt im Bereich von 1 bis etwa 0,5 Vol.-% oder von I bis etwa 0,1 Vol.-% oder weniger liegt, wenn eine Härtungswirkung auf der Basis einer Modifikation der Transformation der Mikrostruktur bereitgestellt wird.

21. Verfahren nach einem der vorangehenden Ansprüche, dadurch gekennzeichnet, daß das Gußeisen oder der Stahl ausgewählt ist aus der Gruppe, die Eisen, Chromeisen, Hochlegierungseisen, Werkzeugstahl, Mittellegierungsstahl, Niederlegierungsstahl, S.G.-Eisen, Stahl oder Gußeisen umfaßt, mit einem Kohlenstoffgehalt, der im Bereich 0,3 bis 3,8 % liegt, und die Stickstoff bis zu 0,1 % enthalten können.

22. Walzwerkwalze mit wenigstens einem äußeren Teil, der ein Gußeisen- oder Stahlprodukt umfaßt, das eine Kohlenstofflegierung mit einer Mikrostruktur umfaßt, die aus Phasentransformation bei Abkühlung hervorgegangen ist und darin dispergiert diskrete Legierungscarbidteilchen aufweist, wobei das Legierungscarbid eine solche Zusammensetzung hat, daß die Dichte des Legierungscarbids, die im Bereich von 6 bis 8 g pro cm³ liegt, mit derjenigen des Gußeisens oder Stahls zusammenpaßt.

23. Walzwerkwalze nach Anspruch 22, dadurch gekennzeichnet, daß die Mikrostruktur eine Matrix und Transformationscarbid umfaßt, die aus Phasentransformation des technischen Eisenmetalls hervorgegangen sind.

24. Walzwerkwalze nach Anspruch 23, dadurch gekennzeichnet, daß die diskreten Legierungscarbidteilchen in der Matrix verteilt sind.

25. Walzwerkwalze nach Anspruch 23 oder Anspruch 24, dadurch gekennzeichnet, daß die diskreten Legierungscarbidteilchen im Transformationscarbid verteilt sind.

26. Walzwerkwalze nach einem der Ansprüche 22 bis 25, dadurch gekennzeichnet, daß die diskreten Legierungscarbidteilchen gleichförmig in der Mikrostruktur verteilt sind.

27. Walzwerkwalze nach einem der vorangehenden Ansprüche, dadurch gekennzeichnet, daß das Legierungscarbid ausgewählt ist aus der Gruppe, die Chrom-, Molybdän-, Titan-, Wolfram-, Niob-, Vanadium- oder Mischcarbide derselben umfaßt, wie etwa Cr₇C₃, (CrMo)₇C₃ oder gemischte Carbonitride derselben.

28. Walzwerkwalze nach einem der vorangehenden Ansprüche, dadurch gekennzeichnet, daß das Carbid ein gemischtes Wolfram-Titan-Carbid der Art (TiW)C ist, wobei das Gewichtsverhältnis von Titan zu Wolfram etwa 1:1 beträgt und vorzugsweise im Verhältnisbereich liegt:
1:1 bis 1:1,17

29. Walzwerkwalze nach einem der vorangehenden Ansprüche, dadurch gekennzeichnet, daß die Legierungscarbidteilchen eine maximale Abmessung von bis zu 10 Mikrometern (10 Mikrons) und vorzugsweise 1-5 Mikrometer (1.5 Mikrons) und bevorzugter 2-5 Mikrometer (2-5 Mikrons) aufweisen.

30. Walzwerkwalze nach einem der vorangehenden Ansprüche, dadurch gekennzeichnet, daß die zugegebene Menge an Legierungscarbidteilchen derart ist, daß bis zu 20 %, vorzugsweise bis zu 5 bis 20 %, volumenbezogen, Legierungscarbidteilchen im festen Metall erreicht werden.

31. Walzwerkwalze nach Anspruch 30, dadurch gekennzeichnet, daß der Legierungscarbidgehalt im Bereich 0,1 bis 20 Vol.-% und bevorzugter 3 bis 10 % liegt, wenn eine Härtungswirkung auf der Basis des Gesetzes der Mischungen bereitgestellt wird.

32. Walzwerkwalze nach Anspruch 30, dadurch gekennzeichnet, daß der Legierungscarbidgehalt im Bereich von 1 bis etwa 0,5 Vol.-% oder von 1 bis etwa 0,1 Vol.-% oder weniger liegt, wenn eine Härtungswirkung auf der Basis einer Modifikation der Transformation der Mikrostruktur bereitgestellt wird.

33. Walzwerkwalze nach einem der vorangehenden Ansprüche, dadurch gekennzeichnet, daß das Gußeisen oder der Stahl ausgewählt ist aus der Gruppe, die Eisen, Chromeisen, Hochlegierungsstahl, Werkzeugstahl, Mittellegierungsstahl, Niederlegierungsstahl, S.G.-Eisen, Stahl oder Gußeisen umfaßt, mit einem Kohlenstoffgehalt, der im Bereich 0,3-3,8 % liegt, und die Stickstoff bis zu 0,1 % enthalten können.

34. Verfahren nach einem der Ansprüche 1 bis 21, dadurch gekennzeichnet, daß die Walzwerkwalze eine Verbundwalzwerkwalze der Art ist, die einen Kern und einen Außenmantel aufweist, mit fakultativ wenigstens einer Zwischenschicht, wobei der Mantel besagten äußeren Teil umfaßt.

35. Walzwerkwalze nach einem der Ansprüche 22 bis 33, dadurch gekennzeichnet, daß die Walzwerkwalze eine Verbundwalzwerkwalze der Art ist, die einen Kern und einen Außenmantel aufweist, mit fakultativ wenigstens einer Zwischenschicht, wobei der Mantel besagten äußeren Teil umfaßt.

36. Verfahren nach Anspruch 34, dadurch gekennzeichnet, daß die Legierungscarbidteilchen in ein geschmolzenes technisches Eisenmetall eingebracht werden, aus der der Mantel hergestellt werden soll, und anschließend das technische Eisenmetall mit den Legierungscarbidteilchen darin in eine Form gegossen wird.

37. Verfahren nach Anspruch 34 oder Anspruch 36, dadurch gekennzeichnet, daß die Verbundwalze durch Schleuderguß hergestellt wird.

38. Verfahren nach einem der Ansprüche 1 bis 21, dadurch gekennzeichnet, daß die Walze hergestellt wird, indem ein Elektroschlacke-Umschmelzprozeß an einer selbstverzehrenden Elektrode durchgeführt wird, die einen Innenkörper umfaßt, der mit einer äußeren Plattierung versehen ist, die ein hohles Element umfaßt, das besagte beschichtete Legierungscarbidteilchen enthält.

39. Verfahren nach Anspruch 38, dadurch gekennzeichnet, daß das hohle Element auch einen Pulverlegierungsbestandteil enthält.

40. Verfahren nach Anspruch 38 oder Anspruch 39, dadurch gekennzeichnet, daß der Elektroschlacke-Umschmelzprozeß durchgeführt wird, um eine Walze bereitzustellen, die einen inneren Teil mit einer ersten Zusammensetzung und einen Oberflächenteil mit einer zweiten Zusammensetzung umfaßt, die verschieden ist von der ersten Zusammensetzung, und das Metall der Walze zwischen dem inneren Teil und dem Oberflächenteil eine Zusammensetzung aufweist, die sich von der ersten Zusammensetzung zur zweiten Zusammensetzung ohne Diskontinuität ändert.

41. Verfahren nach Anspruch 38 oder Anspruch 40, dadurch gekennzeichnet, daß der Elektroschlacke-Umschmelzprozeß durchgeführt wird, um eine Walze mit im wesentlichen gleichförmiger Zusammensetzung über den gesamten Querschnitt der Walze bereitzustellen.

42. Verfahren nach Anspruch 34 oder Anspruch 36, dadurch gekennzeichnet, daß die Walze durch Elektroschlacke-Umschmelzplattierung oder Spritzplattierung hergestellt wird.

43. Verfahren nach einem der Ansprüche 1 bis 21, dadurch gekennzeichnet, daß die Walze durch Monoblockstatikguß durch Füllen einer stationären Form mit einem einzigen Gußeisen oder Stahl hergestellt wird.

44. Verfahren nach einem der Ansprüche 1 bis 21, dadurch gekennzeichnet, daß eine Walze durch ein Doppelgießstatikgußverfahren hergestellt wird.

45. Verfahren nach einem der Ansprüche 34, 36, 37 bis 39 oder Ansprüche 42 bis 44, dadurch gekennzeichnet, daß der Kern schuppenförmiges, kompaktes, vernizuläres oder noduläres Gußeisen oder Stahl umfaßt.

46. Verfahren nach einem der Ansprüche 1 bis 21, dadurch gekennzeichnet, daß es das Gießen eines Gußblockes aus besagtem Metall und anschließendes Schmieden des Gußblockes, um eine geschmiedete Walze bereitzustellen, gefolgt von Wärmebehandlung der geschmiedeten Walze, umfaßt.

47. Walzwerkwalze nach einem der Ansprüche 22 bis 33 oder 35, dadurch gekennzeichnet, daß die Walzwerkwalze eine geschmiedete Walze ist.

## Patentansprüche (Patentansprüche für folgende(n) Vertragsstaat(en): AT, CH, LI, DK, GR, IE, MC, PT)

1. Verfahren zur Herstellung von Gußeisen oder Stahl, welches die Schritte umfaßt, daß zu flüssigem Gußeisen oder Stahl feste Legierungscarbidteilchen zugegeben werden und man danach das Gußeisen oder den Stahl fest werden läßt, wobei die Legierungcarbidteilchen eine Dichte von 6 bis 8 g pro cm³ aufweisen, um mit derjenigen des Gußeisens oder Stahls zusammenzupassen, und die festen Carbidteilchen mit einem Metall beschichtet sind, das zuläßt, daß Benetzung zwischen den Teilchen und dem flüssigen Gußeisen oder Stahl auftritt.

2. Verfahren nach Anspruch 1, dadurch gekennzeichnet, daß das Beschichtungsmetall Eisen umfaßt oder eine Eisen-Kohlenstoff-Legierung oder eine Legierung aus zwei oder mehr Elementen, die ausgewählt sind aus der Gruppe, die Eisen, Nickel, Kupfer, Titan und Kohlenstoff umfaßt, oder Nickel oder Kupfer und übliche Nebenbestandteile, und/oder Stickstoff.

3. Verfahren nach Anspruch 1 oder 2, dadurch gekennzeichnet, daß das Beschichtungsmetall einen Schmelzpunkt besitzt, der innerhalb von ungefähr 20°-30°C der Temperatur des Gußeisens oder Stahls liegt, bei der besagte beschichtete Carbidteilchen zugegeben werden.

4. Verfahren nach einem der vorangehenden Ansprüche, dadurch gekennzeichnet, daß die Legierungscarbidteilchen mit Eisen odei mit einer Eisenlegierung, die-einen niedrigeren Kohlenstoffgehalt aufweist als derjenige des Gußeisens oder Stahls, zu dem sie zugegeben werden, beschichtet werden und die beschichteten Legierungscarbidteilchen zum Gußeisen oder Stahl zugegeben und darin ausreichend lange belassen werden, damit Kohlenstoff aus dem Gußeisen oder Stahl in die Beschichtung hinein diffundiert und so eine Zusammensetzung erzeugt, die einen Schmelzpunkt hat, der mit der Betriebstemperatur des Gußeisens oder Stahls zusammenpaßt.

5. Verfahren nach einem der vorangehenden Ansprüche, dadurch gekennzeichnet, daß die beschichteten Legierungscarbidteilchen zum flüssigen Gußeisen oder Stahl entweder im Schmelzofen oder in einer Pfanne, in die das Metall aus dem Schmelzofen gegossen worden ist, oder im Metallstrom, der aus dem Schmelzofen in die Pfanne gegossen wird, oder im Metallstrom, der aus der Pfanne in eine Form gegossen wird, zugegeben werden.

6. Verfahren nach Anspruch 5, dadurch gekennzeichnet, daß die beschichteten Legierungscarbidteilchen im Schmelzofen zugegeben werden und daß der Schmelzofen ein Induktionsofen ist.

7. Verfahren nach einem der vorangehenden Ansprüche, dadurch gekennzeichnet, daß die beschichteten Legierungscarbidteilchen zum Gußeisen oder Stahl in einer inerten Umgebung zugegeben werden.

8. Verfahren nach einem der vorangehenden Ansprüche, dadurch gekennzeichnet, daß die beschichteten Legierungscarbidteilchen zur Gußeisen- oder Stahlschmelze in der Form eines Pulvers zugegeben werden, das Pulverteilchen mit einer Teilchengröße von bis zu 2 mm und vorzugsweise etwa 500 Mikrometern (500 Mikrons) umfaßt und Legierungscarbidteilchen mit einer Teilchengröße von bis zu 10 Mikrometern (10 Mikrons) und vorzugsweise im Bereich 1-5 Mikrometer (1,5 Mikrons) und bevorzugter 2,5 Mikrometer (2-5 Mikrons) enthält.

9. Verfahren nach einem der vorangehenden Ansprüche, dadurch gekennzeichnet, daß die beschichteten Legierungscarbidteilchen zur Gußeisen- oder Stahlschmelze in der Form eines Pulvers zugegeben werden, wobei die Pulverteilchen umfassen:
| | |
|---|---|
| 25% | Besckichtungsmetall |
| 30% | Ti |
| 35% | W |
| Rest | Eisen und bis zu 3,5 % freien Kohlenstoff und übliche Nebenbestandteile |

10. Verfahren nach einem der vorangehenden Ansprüche, dadurch gekennzeichnet, daß das Beschichtungsmetall vollständig oder im wesentlichen vollständig Alpha-Eisen und bis zu 3,5 % freien Kohlenstoff umfaßt.

11. Verfahren nach einem der Ansprüche 1 bis 8, dadurch gekennzeichnet, daß die beschichteten Legierungscarbidteilchen zur Gußeisen- oder Stahlschmelze in der Form eines Pulvers zugegeben werden, wobei die Pulverteilchen umfassen:
| | |
|---|---|
| 27% | Besckichtungsmetall |
| 30% | Ti |
| 35% | W |
| Rest | Eisen und bis zu 0,5 % freien Kohlenstoff und übliche Nebenbestandteile |

12. Verfahren nach einem der Ansprüche 1 bis 8 oder Anspruch 11, dadurch gekennzeichnet, daß das Beschichtungsmetall eine Legierung aus Eisen, Nickel und Kohlenstoff umfaßt.

13. Verfahren nach Anspruch 12, dadurch gekennzeichnet, daß die Legierung aus Eisen, Nickel und Kohlenstoff umfaßt:
| | |
|---|---|
| 59% | Nickel |
| 41% | Eisen und bis zu 0,5 % freien Kohlenstoff und übliche Nebenbestandteile |

14. Verfahren nach einem der Ansprüche 1 bis 4 oder einem der Ansprüche 8 bis 13, sofern abhängig von einem der Ansprüche 1 bis 4, dadurch gekennzeichnet, daß die beschichteten Legierungscarbidteilchen während eines Elektroschlacke-Umschmelzprozesses zugegeben werden.

15. Verfahren nach einem der vorangehenden Ansprüche, dadurch gekennzeichnet, daß das Legierungscarbid ausgewählt ist aus der Gruppe, die aus Chrom-, Molybdän-, Titan-, Wolfram-, Niob-, Vanadium- oder Mischcarbiden derselben besteht, wie etwa Cr₇C₃, (CrMo)₇C₃ oder gemischten Carbonitriden derselben.

16. Verfahren nach einem der vorangehenden Ansprüche, dadurch gekennzeichnet, daß das Carbid ein gemischtes Wolfram-Titan-Carbid der Art (TiW)C ist, wobei das Gewichtsverhältnis von Titan zu Wolfram etwa 1:1 beträgt und vorzugsweise im Verhältnisbereich liegt:
1:1 bis 1:1.17

17. Verfahren nach einem der vorangehenden Ansprüche, dadurch gekennzeichnet, daß die Legierungscarbidteilchen eine maximale Abmessung von bis zu 10 Mikrometern (10 Mikrons) und vorzugsweise 1-5 Mikrometer (1-5 Mikrons) und bevorzugter 2-5 Mikrometer (2-5 Mikrons) besitzen.

18. Verfahren nach einem der vorangehenden Ansprüche, dadurch gekennzeichnet, daß die zugegebene Menge an Legierungscarbidteilchen derart ist, daß bis zu 20 %, vorzugsweise bis zu 5 bis 20 %, volumenbezogen, Legierungscarbidteilchen im festen Metall erreicht werden.

19. Verfahren nach Anspruch 18, dadurch gekennzeichnet, daß der Legierungscarbidgehalt im Bereich 0,1 bis 20 Vol.-% und bevorzugter 3 bis 10 % liegt, wenn eine Härtungswirkung auf der Basis des Gesetzes der Mischungen bereitgestellt wird.

20. Verfahren nach Anspruch 18, dadurch gekennzeichnet, daß der Legierungscarbidgehalt im Bereich von 0.1 bis etwa 0,5 Vol.-% oder von 1 bis etwa 0,1 Vol.-% oder weniger liegt, wenn eine Härtungswirkung auf der Basis einer Modifikation der Transformation der Mikrostruktur bereitgestellt wird.

21. Verfahren nach einem der vorangehenden Ansprüche, dadurch gekennzeichnet, daß das Gußeisen oder der Stahl ausgewählt ist aus der Gruppe, die Eisen, Chromeisen, Hochlegierungseisen, Werkzeugstahl, Mittellegierungsstahl, Niederlegierungsstahl, S.G.-Eisen, Stahl oder Gußeisen umfaßt, mit einem Kohlenstoffgehalt, der im Bereich 0,3 bis 3,8 % liegt, und die Stickstoff bis zu 0,1 % enthalten können.

22. Gußeisen- oder Stahlprodukt, das eine Eisen-Kohlenstoff-Legierung mit einer Mikrostruktur umfaßt, die aus Phasentransformation bei Abkühlung hervorgegangen ist und darin dispergierte diskrete Legierungscarbidteilchen aufweist, wobei das Legierungscarbid eine solche Zusammensetzung aufweist, daß die Dichte des Legierungscarbids, die im Bereich von 6 bis 8 g pro cm³ liegt, mit derjenigen des Gußeisens oder Stahls zusammenpaßt.

23. Produkt nach Anspruch 22, dadurch gekennzeichnet, daß die Mikrostruktur eine Matrix und ein Transformationscarbid umfaßt, die aus Phasentransformation des Gußeisens oder Stahls hervorgegangen sind.

24. Produkt nach Anspruch 23, dadurch gekennzeichnet, daß die diskreten Legierungscarbidteilchen in der Matrix verteilt sind.

25. Produkt nach Anspruch 23 oder Anspruch 24, dadurch gekennzeichnet, daß die diskreten Legierungscarbidteilchen im Transformationscarbid verteilt sind.

26. Produkt nach einem der Ansprüche 22 bis 25, dadurch gekennzeichnet, daß die diskreten Legierungscarbidteilchen gleichförmig in der Mikrostruktur verteilt sind.

27. Produkt nach einem der vorangehenden Ansprüche, dadurch gekennzeichnet, daß das Legierungscarbid ausgewählt ist aus der Gruppe, die Chrom-, Molybdän-, Titan-, Wolfram-, Niob-, Vanadium- oder Mischcarbide derselben umfaßt, wie etwa Cr₇C₃, (CrMo)7C3 oder gemischte Carbonitride derselben.

28. Produkt nach einem der vorangehenden Ansprüche, dadurch gekennzeichnet, daß das Carbid ein gemischtes Wolfram-Titan-Carbid der Art (TiW)C ist, wobei das Gewichtsverhältnis von Titan zu Wolfram etwa 1:1 beträgt und vorzugsweise im Verhältnisbereich liegt:
1:1 bis 1:1,17

29. Produkt nach einem der vorangehenden Ansprüche, dadurch gekennzeichnet, daß die Legierungscarbidteilchen eine maximale Abmessung von bis zu 10 Mikrometern (10 Mikrons) und vorzugsweise 1-5 Mikrometer (1-5 Mikrons) und bevorzugter 2-5 Mikrometer (2-5 Mikrons) aufweisen.

30. Produkt nach einem der vorangehenden Ansprüche, dadurch gekennzeichnet, daß die zugegebene Menge an Legierungscarbidteilchen derart ist, daß bis zu 20 %, vorzugsweise bis zu 5 bis 20 %, volumenbezogen, Legierungscarbidteilchen im festen Metall erreicht werden.

31. Produkt nach Anspruch 30, dadurch gekennzeichnet, daß der Legierungscarbidgehalt im Bereich 0,1 bis 20 Vol.-% und bevorzugter 3 bis 10 % liegt, wenn eine Härtungswirkung auf der Basis des Gesetzes der Mischungen bereitgestellt wird.

32. Produkt nach Anspruch 30, dadurch gekennzeichnet, daß der Legierungscarbidgehalt im Bereich von 1 bis etwa 0,5 Vol.-% oder von 1 bis etwa 0,1 Vol.-% oder weniger liegt, wenn eine Härtungswirkung auf der Basis einer Modifikation der Transformation der Mikrostruktur bereitgestellt wird.

33. Produkt nach einem der vorangehenden Ansprüche, dadurch gekennzeichnet, daß das Gußeisen oder der Stahl ausgewählt ist aus der Gruppe, die Eisen, Chromeisen, Hochlegierungsstahl, Werkzeugstahl, Mittellegierungsstahl, Niederlegierungsstahl, S.G.-Eisen, Stahl oder Gußeisen umfaßt, mit einem Kohlenstoffgehalt, der im Bereich 0,3-3,8 % liegt, und die Stickstoff bis zu 0,1 % enthalten können.

34. Verfahren zur Herstellung einer Walzwerkwalze, dadurch gekennzeichnet, daß ein Metall, das gemäß einem der Ansprüche 1 bis 21 hergestellt ist, oder ein Metall gemäß einem der Ansprüche 22 bis 33 gegossen wird, um wenigstens einen äußeren Teil der Walzwerkwalze herzustellen.

35. Verfahren nach Anspruch 34, dadurch gekennzeichnet, daß die Walzwerkwalze eine Verbundwalzwerkwalze der Art ist, die einen Kern und einen Außenmantel aufweist, mit fakultativ wenigstens einer Zwischenschicht, wobei der Mantel besagten äußeren Teil umfaßt.

36. Produkt nach einem der Ansprüche 15 bis 19 oder Ansprüche 22 bis 33, dadurch gekennzeichnet, daß das Produkt eine Walzwerkwalze ist.

37. Verfahren nach Anspruch 36, dadurch gekennzeichnet, daß die Walzwerkwalze eine Verbundwalzwerkwalze der Art ist, die einen Kern und einen Außenmantel aufweist, mit fakultativ wenigstens einer Zwischenschicht, wobei der Mantel besagten äußeren Teil umfaßt.

38. Verfahren nach Anspruch 35, dadurch gekennzeichnet, daß die Legierungscarbidteilchen in ein geschmolzenes Gußeisen oder einen geschmolzenen Stahl eingebracht werden, aus dem der Mantel hergestellt werden soll, und anschließend das Gußeisen oder der Stahl mit den Legierungscarbidteilchen darin in eine Form gegossen wird.

39. Verfahren nach Anspruch 35 oder Anspruch 38, dadurch gekennzeichnet, daß die Verbundwalze durch Schleuderguß hergestellt wird.

40. Verfahren nach einem der Ansprüche 1 bis 21, dadurch gekennzeichnet, daß die Walze hergestellt wird, indem ein Elektroschlacke-Umschmelzprozeß an einer selbstverzehrenden Elektrode durchgeführt wird, die einen Innenkörper umfaßt, der mit einer äußeren Plattierung versehen ist, die ein hohles Element umfaßt, das besagte beschichtete Legierungscarbidteilchen enthält.

41. Verfahren nach Anspruch 40, dadurch gekennzeichnet, daß das hohle Element auch einen Pulverlegierungsbestandteil enthält.

42. Verfahren nach Anspruch 40 oder Anspruch 41, dadurch gekennzeichnet, daß der Elektroschlacke-Umschmelzprozeß durchgeführt wird, um eine Walze bereitzustellen, die einen inneren Teil mit einer ersten Zusammensetzung und einen Oberflächenteil mit einer zweiten Zusammensetzung umfaßt, die verschieden ist von der ersten Zusammensetzung, und das Metall der Walze zwischen dem inneren Teil und dem Oberflächenteil eine Zusammensetzung aufweist, die sich von der ersten Zusammensetzung zur zweiten Zusammensetzung ohne Diskontinuität ändert.

43. Verfahren nach Anspruch 40 oder Anspruch 42, dadurch gekennzeichnet, daß der Elektroschlacke-Umschmelzprozeß durchgeführt wird, um eine Walze mit im wesentlichen gleichförmiger Zusammensetzung über den gesamten Querschnitt der Walze bereitzustellen.

44. Verfahren nach Anspruch 34 oder Anspruch 35, dadurch gekennzeichnet, daß die Walze durch Elektroschlacke-Umschmelzplattierung oder Spritzplattierung hergestellt wird.

45. Verfahren nach einem der Ansprüche 1 bis 14 oder Ansprüche 20 bis 26, sofern abhängig von einem der Ansprüche 1 bis 14, dadurch gekennzeichnet, daß die Walze durch Monoblockstatikguß durch Füllen einer stationären Form mit einem einzigen Gußeisen oder Stahl hergestellt wird.

46. Verfahren nach einem der Ansprüche 1 bis 21, dadurch gekennzeichnet, daß eine Walze durch ein Doppelgießstatikgußverfahren hergestellt wird.

47. Verfahren nach einem der Ansprüche 34, 35, 38 bis 41 oder Ansprüche 44 bis 46, dadurch gekennzeichnet, daß der Kem schuppenförmiges, kompaktes, vermizuläres oder noduläres Gußeisen oder Stahl umfaßt.

48. Verfahren nach einem der Ansprüche 1 bis 21, dadurch gekennzeichnet, daß es das Gießen eines Gußblockes aus besagtem Metall und anschließendes Schmieden des Gußblockes, um eine geschmiedete Walze bereitzustellen, gefolgt von Wärmebehandlung der geschmiedeten Walze, umfaßt.

49. Produkt gemäß Anspruch 36, dadurch gekennzeichnet, daß die Walzwerkwalze eine geschmiedete Walze ist.

50. Verfahren nach einem der Ansprüche 1 bis 21, dadurch gekennzeichnet, daß besagtes Gußeisen oder besagter Stahl in eine Zentrifugalgießform gegossen wird und ein Zentrifugalgießvorgang daran durchgeführt wird, um ein zentrifugal gegossenes Produkt bereitzustellen.

51. Produkt nach einem der Ansprüche 22 bis 33, dadurch gekennzeichnet, daß das Produkt ein zentrifugal gegossenes Produkt ist.

## Revendications (Revendications pour l'(les) Etat(s) contractant(s) suivant(s): BE, DE, ES, FR, GB, IT, LU, NL, SE)

1. Procédé de fabrication d'un cylindre de laminoir comprenant les étapes consistant à ajouter à de la fonte ou à de l'acier coulé liquide, des particules de carbure d'alliage solide et permettre par la suite à la fonte ou à l'acier coulé de solidifier, dans lequel les particules de carbure de l'alliage présentent une densité de 6 à 8 mg par cm³ qui correspond à celle de la fonte ou de l'acier coulé et les particules de carbure solide sont enrobées avec un métal qui permet que le mouillage se produise entre les particules et la fonte ou l'acier coulé liquide et à couler ledit métal pour procurer au moins une partie externe du cylindre.

2. Procédé selon la revendication 1, dans lequel le métal d'enrobage comprend un alliage de carbone de fer ou du fer, ou un alliage de deux ou plus éléments choisis dans le groupe comprenant le fer, le nickel, le cuivre, le titane et le carbone, ou le nickel ou le cuivre et les résidus habituels et/ou de l'azote.

3. Procédé selon la revendication 1 ou 2, dans lequel le métal d'enrobage présente une température de fusion qui est à l'intérieur d'approximativement 20°C à 30°C de la température du métal ferreux pour pièces de machine auquel lesdites particules de carbure enrobées sont ajoutées.

4. Procédé selon l'une quelconque des revendications précédentes, dans lequel les particules de carbone de l'alliage sont enrobées de fer ou d'un alliage de fer ayant une teneur en carbone plus faible que celle de la fonte ou de l'acier coulé auquel elles sont ajoutés et les particules de carbure de l'alliage enrobées sont ajoutées à la fonte ou à l'acier coulé et autorisées à séjourner dans celui-ci pendant un temps suffisamment long pour que le carbone provenant de la fonte ou de l'acier coulé puisse diffuser dans l'enrobage et produire ainsi une composition qui présente une température de fusion qui correspond à la température opératoire de la fonte ou de l'acier coulé.

5. Procédé selon l'une quelconque des revendications précédentes, dans lequel les particules de carbure de l'alliage enrobées sont ajoutées à la fonte ou à l'acier coulé liquide soit dans le four de fusion, soit dans une poche de coulé dans laquelle le métal a été versé à partir du four de fusion ou dans le flux d'un métal ayant été versé depuis le four de fusion dans la poche ou dans le flux de métal ayant été versé depuis la poche dans un moule.

6. Procédé selon la revendication 5, dans lequel les particules de carbone de l'alliage enrobées sont ajoutées dans le four de fusion.

7. Procédé selon l'une quelconque des revendications précédentes, dans lequel les particules de carbure de l'alliage enrobées sont ajoutées à la fonte ou à l'acier coulé dans un environnement inerte.

8. Procédé selon l'une quelconque des revendications précédentes, dans lequel les particules de carbure de l'alliage enrobées sont ajoutées à la fonte ou à l'acier coulé fondu sous la forme d'une poudre comprenant des particules de poudre ayant une dimension particulaire allant jusqu'à 2 mm et, de préférence, d'environ 500 µm (500 microns) et contenant des particules de carbure de l'alliage ayant une dimension particulaire allant jusqu'à 10 µm (10 microns) et, de préférence, dans la plage de 1 à 5 µm (1 à 5 microns) et, encore plus préférentiellement, de 2 à 5 µm (2 à 5 microns).

9. Procédé selon l'une quelconque des revendications précédentes, dans lequel les particules de carbure de l'alliage enrobées sont ajoutées à la fonte ou à l'acier coulé fondu sous la forme d'une poudre, dans laquelle les particules de poudre comprennent :
| | |
|---|---|
| 25% | méral d'enrobage |
| 30% | Ti |
| 35% | W |
| Rest | Carbone (incluant jusqu'à 3,5 % de carbone non combiné) et les résidus habituels. |

10. Procédé selon l'une quelconque des revendications précédentes, dans lequel le métal d'enrobage comprend du fer alfa totalement ou sensiblement totalement jusqu'à 3,5 % de carbone non combiné.

11. Procédé selon l'une quelconque des revendications 1 à 8, dans lequel les particules de carbure de l'alliage enrobées sont ajoutées à la fonte ou à l'acier coulé fondu sous la forme d'une poudre, dans laquelle les particules de poudre comprennent :
| | |
|---|---|
| 27% | métal d'enrobage |
| 30% | Ti |
| 35% | W |
| Rest | carbone incluant jusqu'à 0,5 % de carbone non combiné) et les résidus habituels. |

12. Procédé selon l'une quelconque des revendications 1 à 8 ou la revendication il dans lequel le métal d'enrobage comprend un alliage de fer, de nickel et de carbone.

13. Procédé selon la revendication 12, dans lequel l'alliage de fer, de nickel et de carbone comprend :
| | |
|---|---|
| 59% | nickel |
| 41% | fer et jusqu'à 0,5 % de carbone non combiné et de résidus habituels. |

14. Procédé selon l'une quelconque des revendications 1 à 4 ou selon l'une quelconque des revendications 8 à 13 en combinaison avec l'une quelconque des revendications 1 à 4, dans lequel les particules de carbure de l'alliage enrobées sont ajoutées pendant une opération de raffinement sous laitier électroconducteur.

15. Procédé selon l'une quelconque des revendications précédentes, dans lequel le carbure de l'alliage est choisi dans le groupe comprenant le chrome, le molybdène, le titane, le tungstène, le niobium, le vanadium ou leurs carbures mélangés tels que Cr₇C₃, (CrMo)₇C₃ ou leurs carbonitrures mélangés.

16. Procédé selon l'une quelconque des revendications précédentes, dans lequel le carbure est un carbure de titane et de tungstène mélangés du type (TiW)C où le rapport du titane au tungstène est d'environ 1 : 1 en poids et, de préférence, dans la plage des rapports :
1 : 1 à 1 : 1,17.

17. Procédé selon l'une quelconque des revendications précédentes, dans lequel les particules de carbure de l'alliage présentent une dimension maximale allant jusqu'à 10 µm (10 microns) et, de préférence, de 1 à 5 µm (1 à 5 microns) et, encore plus préférentiellement, de 2 à 5 µm (2 à 5 microns).

18. Procédé selon l'une quelconque des revendications précédentes, dans lequel la quantité de particules de carbure de l'alliage ajoutées est telle à pouvoir obtenir jusqu'à 20 %, de préférence jusqu'à 5 à 20 % en volume de particules de carbure de l'alliage dans le métal solide.

19. Procédé selon la revendication 18, dans lequel la teneur en carbure de l'alliage est dans la plage de 0,1 à 20 % en volume et, encore plus préférentiellement, de 3 à 10 % lorsqu'un effet de durcissement sur la base de la loi des mélanges est procuré.

20. Procédé selon la revendication 18, dans lequel la teneur en carbure de l'alliage est dans la plage allant de 1 % à environ 0,5 % en volume ou allant de 1 % à environ 0,1 % en volume ou moins lorsqu'un effet de durcissement basé sur une modification de la transformation de la micro structure est procuré.

21. Procédé selon l'une quelconque des revendications précédentes, dans lequel la fonte ou l'acier coulé est choisi dans le groupe qui est constitué du fer, de la fonte au chrome, de l'acier fortement allié, de l'acier à outils, de l'acier moyennement allié, de l'acier faiblement allié, du fer S.G., de la fonte ou de l'acier coulé ayant une teneur en carbone se trouvant dans la plage de 0,3 à 3,8 % et qui peut contenir de 1'azote jusqu'à 0,1 %.

22. Cylindre de laminoir ayant au moins une partie externe qui comprend un produit de fonte ou d'acier coulé comprenant un alliage de carbone ayant une micro structure qui résulte de la transformation de phase lors du refroidissement et ayant dispersé dans celle-ci des particules de carbure d'alliage discrètes dans lequel le carbure d'alliage a une composition telle que la densité du carbure de l'alliage se trouve dans la plage de 6 à 8mg par cm³ qui correspond à celle de la fonte ou de l'acier coulé.

23. Cylindre de laminoir selon la revendication 22, dans lequel la micro structure comprend une matrice et un carbure de transformation qui résulte de la transformation de phase du métal ferreux pour pièces de machine.

24. Cylindre de laminoir selon la revendication 23, dans lequel les particules de carbure de l'alliage discrètes sont distribuées dans la matrice.

25. Cylindre de laminoir selon la revendication 23 ou la revendication 24, dans lequel les particules de carbure de l'alliage discrètes sont distribuées dans le carbure de transformation.

26. Cylindre de laminoir selon l'une quelconque des revendications 22 à 25, dans lequel les particules de carbure de l'alliage discrètes sont distribuées uniformément dans la micro structure.

27. Cylindre de laminoir selon l'une quelconque des revendications précédentes, dans lequel le carbure de l'alliage est choisi dans le groupe comprenant le chrome, le molybdène, le titane, le tungstène, le niobium, le vanadium ou leurs carbures mélangés tels que Cr₇C₃, (CrMo)₇C₃ ou leurs carbonitrures mélangés.

28. Cylindre de laminoir selon l'une quelconque des revendications précédentes, dans lequel le carbure est un carbure de tungstène et de titane mélangés du type (TiW)C où le rapport du titane au tungstène est d'environ 1 : 1 en poids et, de préférence, dans la plage des rapports :
1 : 1 à 1 : 1,17

29. Cylindre de laminoir selon l'une quelconque des revendications précédentes, dans lequel les particules de carbure de l'alliage présentent une dimension maximale allant jusqu'à 10 µm (10 microns), de préférence de 1 à 5 µm (1 à 5 microns) et, encore plus préférentiellement, de 2 à 5 µm (2 à 5 microns).

30. Cylindre de laminoir selon l'une quelconque des revendications précédentes, dans lequel la quantité de particules de carbure de l'alliage ajoutées est telle à pouvoir obtenir jusqu'à 20 %, de préférence jusqu'à 5 à 20 % en volume de particules de carbure de l'alliage dans le métal solide.

31. Produit selon la revendication 30, dans lequel la teneur en carbure de l'alliage est dans la plage de 0,1 à 20 % en volume et, encore plus préférentiellement, de 3 à 10 % lorsqu'un effet de durcissement basé sur la loi des mélanges est procuré.

32. Cylindre de laminoir selon la revendication 30, dans lequel la teneur en carbure de l'alliage est dans la plage allant de 1 % à environ 0,25 % en volume ou allant de 1 % à environ 0,1 % en volume ou moins lorsqu'un effet de durcissement basé sur une modification de la transformation de la micro structure est procuré.

33. Cylindre de laminoir selon l'une quelconque des revendications précédentes, dans lequel la fonte ou l'acier coulé est choisi dans le groupe qui est constitué du fer, de la fonte au chrome, de l'acier fortement allié, de l'acier à outils, de l'acier moyennement allié, de l'acier faiblement allié, du fer S.G., de la fonte ou de l'acier coulé ayant une teneur en carbone se trouvant dans la plage de 0,3 à 3,8 % et qui peut contenir de l'azote jusqu'à 0,1 %.

34. Procédé selon l'une quelconque des revendications 1 à 21, dans lequel le cylindre de laminoir est un cylindre de laminoir composite du type ayant un noyau et une coquille externe avec, facultativement, au moins une couche intermédiaire, dans laquelle la coquille constitue ladite partie externe.

35. Cylindre de laminoir selon l'une quelconque des revendications 22 à 33, dans lequel le cylindre de laminoir est un cylindre de laminoir composite du type ayant un noyau et une coquille externe avec, facultativement, au moins une couche intermédiaire, dans laquelle la coquille constitue ladite partie externe.

36. Procédé selon la revendication 34, dans lequel les particules de carbone de l'alliage sont introduites dans un métal ferreux pour pièces de machine fondue dont la coquille doit être formée et ensuite le métal ferreux pour pièces de machine ayant les particules de carbure de l'alliage dans celui-ci est versé dans un moule.

37. Procédé selon la revendication 34 ou la revendication 36, dans lequel le cylindre composite est fabriqué par coulée centrifuge.

38. Procédé selon l'une quelconque des revendications 1 à 21, dans lequel le cylindre est fabriqué en effectuant une opération de raffinement sous laitier électroconducteur sur une électrode consommable qui comprend un corps interne muni d'un placage externe comprenant un élément creux contenant lesdites particules de carbure de l'alliage enrobées.

39. Procédé selon la revendication 38, dans lequel l'élément creux contient également un ingrédient de l'alliage sous forme de poudre.

40. Procédé selon la revendication 38 ou la revendication 39, dans lequel l'opération de raffinement sous laitier électroconducteur est effectuée pour procurer un cylindre comprenant une partie interne ayant une première composition et une partie de surface ayant une seconde composition qui est différente de la première composition et le métal du cylindre entre la partie interne et la partie de surface ayant une composition qui change de la première composition à la seconde composition sans discontinuité.

41. Procédé selon la revendication 38 ou la revendication 40, dans lequel l'opération de raffinement sous laitier électroconducteur est effectuée pour procurer un cylindre ayant une composition sensiblement uniforme sur toute la section transversale du cylindre.

42. Procédé selon la revendication 34 ou la revendication 36, dans lequel le cylindre est fabriqué par placage par raffinement sous laitier électroconducteur ou par placage par pulvérisation.

43. Procédé selon l'une quelconque des revendications 1 à 21, dans lequel le cylindre est fabriqué par coulage statique monobloc en remplissant un moule fixe avec seulement de la fonte ou de l'acier coulé.

44. Procédé selon l'une quelconque des revendications 1 à 21, dans lequel un cylindre est fabriqué par un procédé de coulée statique versée deux fois.

45. Procédé selon l'une quelconque des revendications 34, 36, 37 à 39 ou des revendications 42 à 44, dans lequel le noyau est constitué de fonte en flocons, compact, vermiculaire ou nodulaire ou d'acier coulé en flocons, compact, vermiculaire ou nodulaire.

46. Procédé selon l'une quelconque des revendications 1 à 21 comprenant l'étape consistant à couler un lingot dudit métal et à forger ensuite le lingot pour procurer un cylindre forgé suivi par le traitement thermique du cylindre forgé.

47. Cylindre de laminoir selon l'une quelconque des revendications 22 à 33 ou 35 dans lequel le cylindre de laminoir est un cylindre forgé

## Revendications (Revendications pour l'(les) Etat(s) contractant(s) suivant(s): AT, CH, LI, DK, GR, IE, MC, PT)

1. Procédé de fabrication de fonte ou d'acier coulé comprenant les étapes consistant à ajouter à de la fonte ou à de l'acier coulé, des particules de carbure d'alliage solide et permettre par la suite à la fonte ou à l'acier coulé de solidifier dans lequel les particules de carbure de l'alliage présentent une densité de 6 à 8 mg par cm³ qui correspond à celle de la fonte ou de l'acier coulé et les particules de carbure solide sont enrobées avec un métal qui permet que le mouillage se produise entre les particules et la fonte ou l'acier coulé liquide et à couler ledit métal pour procurer au moins une partie externe du cylindre.

2. Procédé selon la revendication 1, dans lequel le métal d'enrobage comprend un alliage de carbone de fer ou du fer, ou un alliage de deux ou plus éléments choieis dans le groupe comprenant le fer, le nickel, le cuivre, le titane et le carbone, ou le nickel ou le cuivre et les résidus habituels et/ou de l'azote.

3. Procédé selon la revendication 1 ou 2, dans lequel le métal de recouvrement ou d'enrobage présente une température de fusion qui est à l'intérieur d'approximativement 20°C à 30°C de la température du métal ferreux pour pièces de machine auquel lesdites particules de carbure enrobées sont ajoutées.

4. Procédé selon l'une quelconque des revendications précédentes, dans lequel les particules de carbone de l'alliage sont enrobées de fer ou d'un alliage de fer ayant une faible teneur en carbone plus faible que celle de la fonte ou de l'acier coulé auquel elles sont ajoutés et les particules de carbure de l'alliage enrobées sont ajoutées à la fonte ou à l'acier coulé et autorisées à séjourner dans celui-ci pendant un temps suffisamment long pour que le carbone provenant de la fonte ou de l'acier coulé puisse diffuser dans l'enrobage et produire ainsi une composition qui présente une température de fusion qui correspond à la température opératoire de la fonte ou de l'acier coulé.

5. Procédé selon l'une quelconque des revendications précédentes, dans lequel les particules de carbure de l'alliage enrobées sont ajoutées à la fonte ou à l'acier coulé liquide soit dans le four de fusion, soit dans une poche de coulé dans laquelle le métal a été versé à partir du four de fusion ou dans le flux d'un métal ayant été versé depuis le four de fusion dans la poche ou dans le flux de métal ayant été versé depuis la poche dans un moule.

6. Procédé selon la revendication 5, dans lequel les particules de carbone de l'alliage enrobées sont ajoutées dans le four de fusion, et dans lequel le four de fusion est un four à induction.

7. Procédé selon l'une quelconque des revendications précédentes, dans lequel les particules de carbure de l'alliage enrobées sont ajoutées à la fonte ou à l'acier coulé dans un environnement inerte.

8. Procédé selon l'une quelconque des revendications précédentes, dans lequel les particules de carbure de l'alliage enrobées sont ajoutées à la fonte ou à l'acier coulé fondu sous la forme d'une poudre comprenant des particules de poudre ayant une dimension particulaire allant jusqu'à 2 mm et, de préférence, d'environ 500 µm (500 microns), et contenant des particules de carbure de l'alliage ayant une dimension particulaire allant jusqu'à 10 µm (10 microns) et, de préférence, dans la plage de 1 à 5 µm (1 à 5 microns) et, encore plus préférentiellement, de 2 à 5 µm (2 à 5 microns).

9. Procédé selon l'une quelconque des revendications précédentes, dans lequel les particules de carbure de l'alliage enrobées sont ajoutées à la fonte ou à l'acier coulé fondu sous la forme d'une poudre, dans laquelle les particules de poudre comprennent :
| | |
|---|---|
| 25% | méral d'enrobage |
| 30% | Ti |
| 35% | W |
| Rest | Carbone (incluant jusqu'à 3,5 % de carbone non combiné) et les résidus habituels. |

10. Procédé selon l'une quelconque des revendications précédentes, dans lequel le métal d'enrobage comprend du fer alfa totalement ou presque totalement, jusqu'à 3,5 % de carbone non combiné.

11. Procédé selon l'une quelconque des revendications 1 à 8, dans lequel les particules de carbure de l'alliage enrobées sont ajoutées à la fonte ou à l'acier coulé fondu sous la forme d'une poudre, dans laquelle les particules de poudre comprennent :
| | |
|---|---|
| 25% | méral d'enrobage |
| 30% | Ti |
| 35% | W |
| Rest | Carbone (incluant jusqu'à 0,5 % de carbone non combiné) et les résidus habituels. |

12. Procédé selon l'une quelconque des revendications 1 à 8 ou la revendication 11, dans lequel le métal d'enrobage comprend un alliage de fer, de nickel et de carbone.

13. Procédé selon la revendication 12, dans lequel l'alliage de fer, de nickel et de carbone comprend
| | |
|---|---|
| 59% | nickel |
| 41% | fer et jusqu'à 0,5 % de carbone non combiné et de résidus habituels. |

14. Procédé selon l'une quelconque des revendications 1 à 4 ou selon l'une quelconque des revendications 8 à 13 en combinaison avec l'une quelconque des revendications 1 à 4, dans lequel les particules de carbure de l'alliage enrobées sont ajoutées pendants une opération de raffinement sous laitier électroconducteur.

15. Procédé selon l'une quelconque des revendications précédentes, dans lequel le carbure de l'alliage est choisi dans le groupe comprenant le chrome, le molybdène, le titane, le tungstène, le niobium, le vanadium ou leurs carbures mélangés tels que Cr₇C₃, (CrMo)₇C₃ ou leurs carbonitrures mélangés.

16. Procédé selon l'une quelconque des revendications précédentes, dans lequel le carbure est un carbure de titane et de tungstène mélangés du type (TiW)C où le rapport du titane au tungstène est d'environ 1 : 1 en poids et, de préférence, dans la plage des rapports :
1 : 1 à 1 : 1,17.

17. Procédé selon l'une quelconque des revendications précédentes, dans lequel les particules de carbure de l'alliage présentent une dimension maximale allant jusqu'à 10 µm (10 microns) et, de préférence, de 1 à 5 µm (1 à 5 microns) et, encore plus préférentiellement, de 2 à 5 µm (2 à 5 microns).

18. Procédé selon l'une quelconque des revendications précédentes, dans lequel la quantité de particules de carbure de l'alliage ajoutées est telle à pouvoir obtenir jusqu'à 20 %, de préférence jusqu'à 5 à 20 % en volume de particules de carbure de l'alliage dans le métal solide.

19. Procédé selon la revendication 18, dans lequel la teneur en carbure de l'alliage est dans la plage de 0,1 à 20 % en volume et, encore plus préférentiellement, de 3 à 10 % lorsqu'un effet de durcissement sur la base de la loi des mélanges est procuré.

20. Procédé selon la revendication 18, dans lequel la teneur en carbure de l'alliage est dans la plage allant de 0,1 % à 0,5 % en volume ou allant de 1 % à environ 0,1 % en volume ou moins lorsqu'un effet de durcissement basé sur une modification de la transformation de la micro structure est procuré.

21. Procédé selon l'une quelconque des revendications précédentes, dans lequel la fonte ou l'acier coulé est choisi dans le groupe qui est constitué du fer, de la fonte au chrome, de l'acier fortement allié, de l'acier à outils, de l'acier moyennement allié, de l'acier faiblement allié, du fer S.G., de la fonte ou de l'acier coulé ayant une teneur en carbone se trouvant dans la plage de 0,3 à 3,8 % et qui peut contenir de l'azote jusqu'à 0,1 %.

22. Produit de fonte ou d'acier coulé comprenant un alliage de carbone ayant une micro structure qui résulte de la transformation de phase lors du refroidissement et ayant dispersé dans celle-ci des particules de carbure de l'alliage discrètes, dans lequel le carbure de l'alliage a une composition telle que la densité du carbure de l'alliage se trouve dans la plage de 6 à 8mg par cm³ qui correspond à celle de la fonte ou de l'acier coulé.

23. Produit selon la revendication 22, dans lequel la micro structure comprend une matrice et un carbure de transformation qui résulte de la transformation de phase de la fonte ou de l'acier coulé.

24. Produit selon la revendication 23, dans lequel les particules de carbure de l'alliage discrètes sont distribuées dans la matrice.

25. Produit selon la revendication 23 ou la revendication 24, dans lequel les particules de carbure de l'alliage discrètes sont distribuées dans le carbure de transformation.

26. Produit selon l'une quelconque des revendications 22 à 25, dans lequel les particules de carbure de l'alliage discrètes sont distribuées uniformément dans la micro structure.

27. Produit selon l'une quelconque des revendications précédentes, dans lequel le carbure de l'alliage est choisi dans le groupe comprenant le chrome, le molybdène, le titane, le tungstène, le niobium, le vanadium ou leurs carbures mélangés tels que Cr₇C₃, (CrMo)₇C₃ ou leurs carbonitrures mélangés.

28. Produit selon l'une quelconque des revendications précédentes, dans lequel le carbure est un carbure de tungstène et de titane mélangés du type (TiW)C où le rapport du titane au tungstène est d'environ 1 : 1 en poids et, de préférence, dans la plage des rapports :
1 : 1 à 1 : 1,17

29. Produit selon l'une quelconque des revendications précédentes, dans lequel les particules de carbure de l'alliage présentent une dimension maximale allant jusqu'à 10 µm (10 microns), de préférence de 1 à 5 µm (1 à 5 microns) et, encore plus préférentiellement, de 2 à 5 µm (2 à 5 microns).

30. Produit selon l'une quelconque des revendications précédentes, dans lequel la quantité de particules de carbure de l'alliage ajoutées est telle à pouvoir obtenir jusqu'à 20 %, de préférence, jusqu'à 5 à 20 % en volume de particules de carbure de l'alliage dans le métal solide.

31. Produit selon la revendication 30, dans lequel la teneur en carbure de l'alliage est dans la plage de 0,1 à 20 % en volume et, encore plus préférentiellement, de 3 à 10 % lorsqu'un effet de durcissement basé sur la loi des mélanges est procuré.

32. Produit selon la revendication 30, dans lequel la teneur en carbure de l'alliage est dans la plage allant de 1 % à environ 0,25 % en volume ou allant de 1 % à environ 0,1 % en volume ou moins lorsqu'un effet de durcissement basé sur une modification de la transformation de la micro structure est procuré.

33. Produit selon l'une quelconque des revendications précédentes, dans lequel la fonte ou l'acier coulé est choisi dans le groupe qui est constitué du fer, de la fonte au chrome, de l'acier fortement allié, de l'acier à outils, de l'acier moyennement allié, de l'acier faiblement allié, du fer S.G., de la fonte ou de l'acier coulé ayant une teneur en carbone se trouvant dans la plage de 0,3 à 3,8 % et qui peut contenir de l'azote jusqu'à 0,1 %.

34. Procédé de fabrication d'un cylindre de laminoir, dans lequel le métal fabriqué selon l'une quelconque des revendications 1 à 21 ou un métal selon l'une quelconque des revendications 22 à 33 est coulé pour fabriquer au moins une partie externe du cylindre de laminoir.

35. Procédé selon la revendication 34, dans lequel le cylindre de laminoir est un cylindre de laminoir composite du type ayant un noyau et une coquille externe avec, facultativement, au moins une couche intermédiaire, dans lequel la coquille constitue ladite partie externe.

36. Produit selon l'une quelconque des revendications 15 à 19 ou des revendications 22 à 33, dans lequel le produit est un cylindre de laminoir.

37. Produit selon la revendication 36, dans lequel le cylindre de laminoir est un cylindre de laminoir composite du type ayant un noyau et une coquille externe avec, facultativement, au moins une couche intermédiaire, dans lequel la coquille constitue ladite partie externe.

38. Procédé selon la revendication 35, dans lequel les particules de carbone de l'alliage sont introduites dans la fonte ou l'acier coulé, dont la coquille doit être formée, et ensuite, la fonte ou l'acier coulé ayant les particules de carbure de l'alliage dans celui-ci est versé dans un moule.

39. Procédé selon la revendication 35 ou la revendication 38, dans lequel le cylindre composite est fabriqué par coulée centrifuge.

40. Procédé selon l'une quelconque des revendications 1 à 21, dans lequel le cylindre est fabriqué en effectuant une opération de raffinement sous laitier électroconducteur sur une électrode consommable qui comprend un corps interne muni d'un placage externe comprenant un élément creux contenant lesdites particules de carbure de l'alliage enrobées.

41. Procédé selon la revendication 40, dans lequel l'élément creux contient également un ingrédient de l'alliage sous forme de poudre.

42. Procédé selon la revendication 40 ou la revendication 41, dans lequel l'opération de raffinement sous laitier électroconducteur est effectuée pour procurer un cylindre comprenant une partie interne ayant une première composition et une partie de surface ayant une seconde composition qui est différente de la première composition et le métal du cylindre entre la partie interne et la partie de surface ayant une composition qui change de la première composition à la seconde composition sans discontinuité.

43. Procédé selon la revendication 40 ou la revendication 42, dans lequel l'opération de raffinement sous laitier électroconducteur est effectuée pour procurer un cylindre ayant une composition sensiblement uniforme sur toute la section transversale du cylindre.

44. Procédé selon la revendication 34 ou la revendication 35, dans lequel le cylindre est fabriqué par placage par raffinement sous laitier électroconducteur ou par placage par pulvérisation.

45. Procédé selon l'une quelconque des revendications 1 à 14 ou des revendications 20 à 26, dans lequel le cylindre est fabriqué par coulage statique monobloc en remplissant un moule fixe avec seulement de la fonte ou de l'acier coulé.

46. Procédé selon l'une quelconque des revendications 1 à 21, dans lequel un cylindre est fabriqué par un procédé de coulée statique versée deux fois.

47. Procédé selon l'une quelconque des revendications 34, 35, 38 à 41 ou des revendications 44 à 46, dans lequel le noyau est constitué de fonte en flocons, compact, vermiculaire ou nodulaire ou d'acier coulé en flocons, compact, vermiculaire ou nodulaire.

48. Procédé selon l'une quelconque des revendications 1 à 21 comprenant l'étape consistant à couler un lingot dudit métal et à forger ensuite le lingot pour procurer un cylindre forgé suivi par le traitement thermique du cylindre forgé.

49. Produit selon la revendication 36, dans lequel le cylindre de laminoir est un cylindre forgé

50. Procédé selon l'une quelconque des revendications 1 à 21, dans lequel ladite fonte ou ledit acier coulé est versé dans un moule à coulée centrifuge et une opération de coulée centrifuge est effectuée sur celui-ci pour procurer un produit coulé par centrifugation.

51. Produit selon l'une quelconque des revendications 22 à 33, dans lequel le produit est un produit coulé de manière centrifuge.
